



US006599684B2

(12) **United States Patent**  
Reynolds et al.

(10) **Patent No.:** **US 6,599,684 B2**  
(45) **Date of Patent:** **Jul. 29, 2003**

(54) **COLOR PHOTOTHERMOGRAPHIC ELEMENT COMPRISING A DYE-FORMING SYSTEM FOR FORMING A NOVEL INFRARED DYE**

(75) Inventors: **James H. Reynolds**, Rochester, NY (US); **Leif P. Olson**, Rochester, NY (US); **Wojciech K. Slusarek**, Rochester, NY (US); **David H. Levy**, Rochester, NY (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/928,834**

(22) Filed: **Aug. 13, 2001**

(65) **Prior Publication Data**

US 2003/0073044 A1 Apr. 17, 2003

(51) **Int. Cl.** <sup>7</sup> ..... **G03C 1/58**; G03C 1/42; G03C 5/16

(52) **U.S. Cl.** ..... **430/350**; 430/21; 430/404; 430/405; 430/442; 430/505; 430/556; 430/558; 430/617; 430/944

(58) **Field of Search** ..... 430/566, 558, 430/944, 505, 21, 510, 617, 404, 405, 442,

(56) **References Cited**

**U.S. PATENT DOCUMENTS**

5,248,739 A 9/1993 Schmidt et al.  
5,415,981 A 5/1995 Clarke et al.  
5,756,269 A 5/1998 Ishikawa et al.

**FOREIGN PATENT DOCUMENTS**

JP 4-86658 \* 3/1992 ..... G03C/8/40  
JP 133947 A 5/2001

\* cited by examiner

*Primary Examiner*—Thorl Chea

(74) *Attorney, Agent, or Firm*—Chris P. Konkol

(57) **ABSTRACT**

The present invention is directed to a photothermographic element comprising at least one imaging layer with a pyrrolotriazole coupler and a developing agent, or precursor thereof, the combination of which is capable of forming an image record in the infrared region of the light spectrum in response to a selected hue of visible light. This expedient leads to the formation of high quality images, especially when scanning photothermographic elements in which the silver halide, metallic silver, and/or any organic silver salts have not been removed. Also disclosed is a method for photothermographically forming a developed image comprising an infrared image record.

**27 Claims, No Drawings**

**COLOR PHOTOTHERMOGRAPHIC  
ELEMENT COMPRISING A DYE-FORMING  
SYSTEM FOR FORMING A NOVEL  
INFRARED DYE**

**FIELD OF THE INVENTION**

The present invention is directed to a color photothermographic element comprising a pyrrolotriazole coupler in reactive association with a hue-shifting phenylenediamine developing agent, or precursor thereof, enabling the formation of an infrared imaging dye in response to visible light of a preselected hue.

**BACKGROUND OF THE INVENTION**

U.S. Pat. No. 5,756,269 to Ishikawa et al. discloses the combination of three different developers with three different couplers. For example, a coupler "Y-1" is used with a hydrazide developing agent to form a yellow dye. Ishikawa et al. does not mention, nor attach any significance to, the fact that the same coupler is a magenta dye-forming coupler if used with a common phenylenediamine developing agent.

Clarke et al., in U.S. Pat. Nos. 5,415,981 and 5,248,739, showed that azo dyes formed from a blocked hydrazide developer are shifted to shorter wavelengths. This is perhaps not surprising since azo dyes derived from "magenta couplers" are known to be typically yellow and are used as masking couplers. The substitution pattern on the masking coupler is such that it can undergo further reaction with the oxidized form of a paraphenylenediamine developer to form a magenta dye.

Infrared dyes are used in the photographic area for certain applications. For example, motion picture soundtracks are typically an optically encoded signal that can be read by an infrared detector during projection. In many instances, this signal is encoded by developed metallic silver. However, some applications use an infrared dye for this signal so that the soundtrack can be developed in a chromogenic photographic developing process. The sound track technology is described by: Ciurca, et al. U.S. Pat. No. 4,178,183; Sakai, et al., U.S. Pat. No. 4,208,210; Osborn, et al., U.S. Pat. No. 4,250,251; Fernandez, et al., U.S. Pat. No. 4,233,389; Monbaliu, et al., U.S. Pat. No. 4,839,267 and Olbrecht, et al. U.S. Pat. Nos. 5,030,544 and 5,688,959. Hawkins, et al. in U.S. Pat. No. 5,842,063 describes the use of non-visible color layers to carry collateral information such as sound or metadata in still pictorial images.

**PROBLEM TO BE SOLVED BY THE PRESENT  
INVENTION**

It has become desirable to limit the amount of solvent or processing chemicals used in the processing of silver-halide films. A traditional photographic processing scheme for color film involves development, fixing, bleaching, and washing, each step typically involving immersion in a tank holding the necessary chemical solution. Images are then produced by optical printing. By scanning the film image following development, some of the processing solutions subsequent to development could be eliminated for the purposes of obtaining a color image. Instead, the scanned image could be used to directly provide the final image to the consumer.

By the use of photothermographic film, it would be possible to eliminate processing solutions altogether, or alternatively, to minimize the amount of processing solu-

tions and the complex chemicals contained therein. A photothermographic (PTG) film by definition is a film that requires energy, typically heat, to effectuate development. A dry PTG film requires only heat; a solution-minimized PTG film may require small amounts of aqueous alkaline solution to effectuate development, which amounts may be only that required to swell the film without excess solution. Development is the process whereby silver ion is reduced to metallic silver and, in a color system, a dye is created in an image-wise fashion.

In PTG films, the silver metal and silver halide is typically retained in the coating after the heat development. It can be difficult to scan through imagewise exposed and photochemically processed silver-halide films when the undeveloped silver halide is not removed from the film during processing. The retained silver halide is reflective, and this reflectivity appears as density in a scanner. The retained silver halide scatters light, decreasing sharpness and raising the overall density of the film, to the point in high-silver films of making the film unsuitable for scanning. High densities result in the introduction of Poisson noise into the electronic form of the scanned image, and this in turn results in decreased image quality. The high density can also increase the time required to scan a given image. If, on the other hand, a scanner is designed with a more powerful light source in order to negate the effects of the film turbidity, scanner cost is increased. In addition, the high reflectivity of a retained silver film can cause reflection of light back in the light source of the scanner, which can degrade the uniformity of the scanner illumination system or cause increased flare.

It is therefore an object of the present invention to improve the scanning of photothermographic film without removing the silver halide and/or metallic silver, or partially removing the same.

**SUMMARY OF THE INVENTION**

It has been found that the scattering and reflectivity of retained silver halide is quite dependent on wavelength, and that blue light is more reflected than green light which in turn is more reflected than red light which in turn is more reflected than infrared light. Accordingly, the practice of forming at least one image record in the infrared leads to lower scattering and higher quality images. Further details of the advantages of scanning in the infrared have been discussed by Szajewski in commonly assigned co-pending U.S. application Ser. No. 09/855,046. However, applying the method of forming infrared dyes disclosed therein to color photothermographic (PTG) films has been found to produce relatively inferior results. In order to effectively practice photothermographic imaging using an infrared absorbing dye component, the  $\lambda_{max}$  of the infrared dye must be significantly separated from the nearest other dye, typically a red absorbing dye. Furthermore, the amount of infrared dye formed under thermal processing conditions must be sufficient that good imaging properties are attainable. It has now been discovered that the use of a certain class of cyan couplers in combination with a hue-shifting developer provides significantly improved infrared dye performance in photothermographic elements. In particular, a surprising and significant increase in the  $\lambda_{max}$  is obtained with the pyrrolotriazole compounds of this invention, compared to the use of a commonly employed cyan dye-forming coupler with a comparable developer.

In a typical film, the blue record offers the highest challenge for scanning. This results from three sources: (1)

as mentioned above, the physics of light scatter indicate that the highest degree of scatter occurs in the blue region of the visible spectrum; (2) the most commonly used silver halide crystal for photographic films are composed of silver bromide with small concentrations of silver iodide, a composition that absorbs significant blue light; (3) because of the intrinsic sensitivity produced by (2), it is common to use a yellow filter record below the blue record that prevents sensitivity of the green and red records to blue light, and this filter layer itself produces addition density in the blue region of the spectrum. As a result, any technology that could avoid use of blue absorbance as a means of reading out image information on the film would substantially improve the ease of film scanning.

In one particular embodiment of the present invention, a pyrrolotriazole type of dye-forming coupler is used to form an infrared dye in at least one color record of a color photothermographic element, in reactive association with a blocked para-phenylenediamine developer containing a substituent in both the 2- and 6-positions (ortho, ortho) relative to the coupling nitrogen atom. Such developers when oxidized yield infrared dyes with such couplers. With conventional developers, such as those used in the C-41 process, these same couplers would yield a cyan dye rather than an infrared dye.

In another embodiment of the present invention, a color photothermographic element comprises a blue light-sensitive layer unit having a pyrrolotriazole-type infrared absorbing dye-forming coupler according to the present invention in combination with a green-light-sensitive layer unit having a magenta dye-forming coupler and a red-light-sensitive layer unit having a cyan dye-forming coupler. In another embodiment of the invention, a photothermographic color element comprises a blue-light-sensitive layer unit having a far-infrared dye-forming agent according to the present invention in combination with a red-light-sensitive layer unit having a pyrrolotriazole near-infrared dye-forming agent, and a green-light-sensitive layer unit having a cyan dye-forming chemistry. By the term "infrared dye" is meant a dye that absorbs in the infrared region as explained below. Further, this invention describes the use of such an infrared dye system in a thermally processable system or other incorporated-developer photographic element, and methods of forming an image using such systems. The invention is also directed to a method of processing photographic or photothermographic films.

#### DETAILED DESCRIPTION OF THE INVENTION

As indicated above, the present invention is directed to a color photothermographic element such as film in which at least one layer comprises a pyrrolotriazole dye-forming coupler, in reactive association a developing agent (or precursor thereof) the combination of which coupler and developer forms an imaging dye in the infrared region of the light spectrum. In particular, the pyrrolotriazole dye-forming coupler is a "typically cyan dye-forming coupler" that is hue shifted to the infrared region. In one embodiment, this is accomplished by using a para-phenylene diamine developer containing substituents, preferably a methyl group, in both the 2- and 6-positions (ortho, ortho) relative to the coupling nitrogen along with selected cyan dye-forming couplers. By the term "typically cyan dye-forming coupler" is meant that the coupler forms a cyan dye with an oxidized form of the conventional developer 4-(N-ethyl-N-2-hydroxyethyl)-2-methylphenylenediamine.

In a preferred embodiment, a photothermographic element according to the present invention comprises blue

recording layer unit (BU) containing at least one dye image-forming coupler, a green recording layer unit (GU) containing at least one dye image-forming coupler, and a red recording layer unit (RU) containing at least one dye image-forming coupler, with the proviso that at least one (preferably all) of the imaging layers in at least one of the BU, GU and RU contains an pyrrolotriazole infrared dye-forming coupler. Any convenient combination of conventional dye image-forming couplers can be employed, so long as the images formed in the distinct film color records or units are distinguishable by the scanner at scanning. Distinct infrared dye-forming couplers can be employed in distinct units to carry distinct color records, as for example a near infrared dye-forming coupler in one of BU, GU or RU and a far infrared dye-forming coupler in another of BU, GU or RU. Conventional dye image-forming couplers are illustrated by *Research Disclosure I*, cited above, X. Dye image formers and modifiers, B. Image-dye-forming couplers.

As indicated above, one embodiment of the present invention involves a photothermographic film comprising at least one blue-light sensitive layer or color unit comprising an infrared dye-forming pyrrolotriazole coupler. Optionally, the PTG film can further comprise a red-light sensitive imaging layer or color unit comprising a cyan dye-forming coupler and a green-light sensitive imaging layer or color unit comprising a magenta dye-forming coupler. Other permutations of known dye forming couplers and color layer light sensitivity can be employed so long as at least one layer comprises a pyrrolotriazole coupler that forms dyes in the infrared region.

A color recording layer unit ("unit" or "color unit") can comprise one or more imaging layers, for example, three imaging layers, which layers are sensitive to the same color. Thus, any one or all of the imaging layers in a color unit can comprise an infrared dye-forming coupler.

Non-infrared imaging layers can be made using art known materials, for example magenta and cyan dye forming couplers with a blocked form of a conventional developing agent or para-phenylenediamine compound. These are typically 4-N,N-dialkylaminoanilines and 2-alkyl-4-N,N-dialkylaminoanilines.

Still another embodiment of the present invention, a light-sensitive color photothermographic element comprises at least one blue light-sensitive layer or unit comprising a magenta dye-forming coupler, at least one green light sensitive layer or unit having a cyan dye-forming coupler, and at least one red light-sensitive layer having an infrared dye-forming coupler. This can be accomplished by employing conventional yellow, magenta and cyan dye forming couplers in combination with an appropriate hue shifting developing agent, for example, of the para-phenylene diamine type. These are typically 2,6-dialkyl-4N,N-dialkylaminoanilines. Examples are described in commonly-assigned copending U.S. Ser. No. 09/931,357 and U.S. Ser. No. 09/871,310, both of which applications are hereby incorporated by reference.

In yet another embodiment of the present invention, a light-sensitive photothermographic color element comprises (at least one) blue light-sensitive layer or unit comprising a cyan dye-forming coupler, a green light-sensitive layer or unit comprising a near infrared dye-forming coupler, and a red light-sensitive layer or unit having a far infrared dye forming coupler. This can be accomplished by using art known magenta, cyan and infrared dye forming couplers in combination with a hue shifting para-phenylene diamine developer, for example, 2,6-dialkyl-4-N,N-dialkylaminoanilines.

It has been found that shifting of a colored dye hue to the infrared, according to the present invention, results in images that are easier to scan since there is less light reflection and scatter during scanning of the film despite the presence of silver halide in the film.

The coupler-developer combination according to the present invention, in which the developer is preferably blocked or otherwise a developer precursor, can be used in a thermally-processable system wherein the incorporated developer chosen for each color-forming record need not be identical in structure, but are chosen to utilize the optimal developer-coupler combination. Thus, the invention encompasses the possible use of one or more different couplers and a number of different developing agents. There can be two different couplers, including one, two, or three different couplers in the same imaging element. It is possible to have more than three couplers, for example, per the Japanese kokai mentioned above. It is also possible to have more than three different developers (or blocked developers), three different developers (or blocked developers), two different developers (or blocked developers), or a single developer (or blocked developer).

In a preferred variant, the photothermographic element is imagewise exposed and developed by dry heat treatment. In another variant of the invention, an imagewise exposed photothermographic element is developed by treatment with, in addition to heat, a chemical base, either by contacting the element to a pH controlling solution or by contacting the element to a pH controlling laminate.

As indicated above, the photothermographic imaging element preferably comprises a blocked form of a developer that results in an infrared dye being formed when the oxidized form of the developer is reacted with the pyrrole-triazole coupler according to the present invention. Preferably, the developer is the neutral or photographically acceptable salt form of the compound represented by the following Structure I:



R<sup>1</sup>, R<sup>2</sup>, R<sup>3</sup>, R<sup>4</sup>, R<sup>5</sup> and R<sup>6</sup> which can be the same or different are individually H, alkyl, substituted alkyl, alkenyl, substituted alkenyl, aryl, substituted aryl, halogen, cyano, hydroxy, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of R<sup>1</sup>, R<sup>2</sup>, R<sup>3</sup>, R<sup>4</sup>, R<sup>5</sup> and R<sup>6</sup> together further form a substituted or unsubstituted carbocyclic or heterocyclic ring structure. In one embodiment, either or both R<sup>3</sup> and R<sup>5</sup>, and R<sup>4</sup> and R<sup>6</sup> form cycloaliphatic six-membered rings. In a preferred embodiment, the developing agent is according to the above formula, with the further proviso that neither R<sup>1</sup> nor R<sup>2</sup> can be H.

Preferably, R<sup>1</sup> and R<sup>2</sup> is a substituted or unsubstituted alkyl or alkoxy or an alkylsulfonamido, more preferably a

C1 to C4 alkyl or alkoxy. Most preferably, the alkyl is an n-alkyl substituent. Preferably, R<sup>3</sup> and R<sup>4</sup> are hydrogen. Preferably, R<sup>5</sup> and R<sup>6</sup> are independently hydrogen or a substituted or unsubstituted alkyl group. R<sup>5</sup> and R<sup>6</sup> may be connected to form a cycloaliphatic ring.

More preferably, the (unblocked) developer is the neutral or photographically acceptable salt form of the compound represented by the following Structure II:



wherein R<sup>1</sup> and R<sup>2</sup> are as described above.

In another preferred embodiment, a blocked developing agent releases a developer in neutral or salt form having the following structure:



I  
wherein R<sub>1</sub> and R<sub>2</sub> is independently an alkyl or hydrogen substituent, preferably both hydrogen, and W<sub>1</sub> and W<sub>2</sub> is 40 either absent or represents the atoms necessary to form a substituted or unsubstituted 5 or 6-membered cycloaliphatic ring, wherein at least one of W<sub>1</sub> and W<sub>2</sub> is present in the above structure. Typical substituents are C1 to C4 alkyl and halogen.

45 A specific example of a developing agent, that is useful in the present invention, preferably in blocked form, either in neutral or salt form, is represented by the following Structure III:



Preferably, at least one other color unit layer, more preferably two other color unit layers, contains a second developer which is also a phenylenediamine developer that, however, differs from that of structure III.

Some specific examples of such other developers include, but are not limited, to N,N-diethyl-p-phenylenediamine,

4-N,N-diethyl-2-methylphenylenediamine, 4-(N-ethyl-N-2-methanesulfonylaminoethyl)-2-methylphenylenediamine, 4-(N-ethyl-N-2-hydroxyethyl)-2-methylphenylenediamine, 4-N,N-diethyl-2-

methanesulfonylaminoethylphenylenediamine, 4-(N-ethyl-N-2-methoxyethyl)-2-methylphenylenediamine, 4,5-dicyano-2-isopropylsulfonylhydrazinobenzene and 4-amino-2,6-dichlorophenol. *The Theory of the Photographic Process*, 4th ed., T. H. James, ed., Macmillan, New York 1977 at pages 291 through 403, the disclosures of which are incorporated by reference, discloses some specific developers useful in the practice of this invention. Other useful developers and developer precursors are disclosed by Hunig et al, *Angew. Chem.*, 70, page 215-ff (1958), by Schmidt et al, U.S. Pat. No. 2,424,256, Pelz et al, U.S. Pat. No. 2,895,825, Wahl et al, U.S. Pat. No. 2,892,714, Clarke et al, U.S. Pat. Nos. 5,284,739 and 5,415,981, Takeuchi et al, U.S. Pat. No. 5,667,945, and Nabeta U.S. Pat. No. 5,723,277 the disclosures of which are incorporated by reference.

As used herein and throughout the specification unless where specifically stated otherwise, the term "alkyl" refers to an unsaturated or saturated, straight or branched chain alkyl group, including alkenyl and aralkyl, and includes cyclic alkyl groups, including cycloalkenyl, and the term "aryl" includes specifically fused aryl.

When reference in this application is made to a particular moiety, or group, this means that the moiety may itself be unsubstituted or substituted with one or more substituents (up to the maximum possible number). For example, "alkyl" or "alkyl group" refers to a substituted or unsubstituted alkyl, while "aryl group" refers to a substituted or unsubstituted benzene (with up to five substituents) or higher aromatic systems. Generally, unless otherwise specifically stated, substituent groups usable on molecules herein include any groups, whether substituted or unsubstituted, which do not destroy properties necessary for the photographic utility of the compound, whether coupler utility or otherwise. Examples of substituents on any of the mentioned groups can include known substituents, such as: halogen, for example, chloro, fluoro, bromo, iodo; alkoxy, particularly those "lower alkyl" (that is, with 1 to 6 carbon atoms), for example, methoxy, ethoxy; substituted or unsubstituted alkyl, particularly lower alkyl (for example, methyl, trifluoromethyl); thioalkyl (for example, methylthio or ethylthio), particularly either of those with 1 to 6 carbon atoms; substituted and unsubstituted aryl, particularly those having from 6 to 20 carbon atoms (for example, phenyl); and substituted or unsubstituted heteroaryl, particularly those having a 5 or 6-membered ring containing 1 to 3 heteroatoms selected from N, O, or S (for example, pyridyl, thienyl, furyl, pyrrolyl); acid or acid salt groups such as any of those described below; and others known in the art. Alkyl substituents may specifically include "lower alkyl" (that is, having 1-6 carbon atoms), for example, methyl, ethyl, and the like. Further, with regard to any alkyl group or alkylene group, it will be understood that these can be branched, unbranched or cyclic.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups. Generally, unless indicated otherwise, alkyl, aryl, and other carbon-containing groups and substituents thereof may include those having up to 48 carbon atoms, typically 1 to 36 carbon atoms and usually less than 24 carbon atoms, but greater numbers are possible depending on the particular substituents selected. For example, ballast groups for couplers will tend to have more carbon atoms than other groups on the coupler.

In general, the pyrrolotriazole couplers used in the present invention for forming an infrared image dye, in combination with a suitable phenylenediamine developer are represented by the following structures (IV) to (VII):



25 The couplers of formula (V) are preferred. In formulas (IV) to (VII), R<sup>7</sup>, R<sup>8</sup> and R<sup>9</sup> each represents a hydrogen atom or a substituent group. The substituent groups represented by R<sup>7</sup>, R<sup>8</sup> and R<sup>9</sup> include an alkyl group, an acyl group, a cyano group, a nitro group, an aryl group, a heterocyclic group, an alkoxy carbonyl group, an aryloxycarbonyl group, a carbamoyl group, a sulfamoyl group, an alkylsulfonyl group or an arylsulfonyl group, any of which may have a substituent group. The substituent groups which R<sup>7</sup>, R<sup>8</sup> and R<sup>9</sup> may have include various substituent groups such as alkyl, cycloalkyl, alkenyl alkynyl, aryl, heterocyclic, alkoxy, aryloxy, cyano, acylamino, sulfonamido, carbamoyl, sulfamoyl, alkoxy carbonyl, aryloxycarbonyl, alkylamino, arylamino, hydroxyl and sulfo groups and halogen atoms. Preferred examples of R<sup>7</sup>, R<sup>8</sup> and R<sup>9</sup> include acyl, cyano, carbamoyl and alkoxy carbonyl groups.

30 35 40 45 50 55 60 65 The group Y is a hydrogen atom or a group which is removable by the coupling reaction with a developing agent oxidant. Examples of the groups represented by Y functioning as anionic removable groups of the 2-equivalent couplers include halogen atoms (for example, chlorine and bromine), an aryloxy group (for example, phenoxy, 4-cyanophenoxy or 4-alkoxycarbonylphenyl), an alkylthio group (for example, methylthio, ethylthio or butylthio), an arylthio group (for example, phenylthio or tolylthio), an alkylcarbamoyl group (for example, methyl-carbamoyl, dimethylcarbamoyl, ethylcarbamoyl, diethyl-carbamoyl, dibutylcarbamoyl, piperidylcarbamoyl or morpholylcarbamoyl), an arylcarbamoyl group (for example, phenylcarbamoyl, methylphenylcarbamoyl, ethylphenylcarbamoyl

or benzylphenylcarbamoyl), a carbamoyl group, an alkylsulfamoyl group (for example, methylsulfamoyl, dimethylsulfamoyl, ethylsulfamoyl, diethylsulfamoyl, dibutylsulfamoyl, piperidylsulfamoyl or morpholylsulfamoyl), an arylsulfamoyl group (for example, phenylsulfamoyl, methylphenylsulfamoyl, ethylphenylsulfamoyl or benzylphenylsulfamoyl), a sulfamoyl group, a cyano group, an alkylsulfonyl group (for example, methanesulfonyl or ethanesulfonyl), an arylsulfonyl group (for example, phenylsulfonyl, 4-chlorophenylsulfonyl or p-toluenesulfonyl), an alkylcarbonyloxy group (for example, acetoxy, propionyloxy or butyroyloxy), an arylcarbonyloxy group (for example, benzoxyloxy, tolyloxy or anisoyloxy) and a nitrogen-containing heterocyclic group (for example, imidazolyl or benzotriazolyl).

The group Z represents a hydrogen atom or a group capable of being released upon color development. The group represented by Z includes the group capable of being released under an alkaline condition as described, for example, in JP-A-61-22844. Z is preferably a hydrogen atom.

Preferred examples of the pyrrolotriazole couplers represented by general Formulas (IV) to (VII) include couplers in each of which at least one of R<sup>7</sup> and R<sup>8</sup> is an electron attractive group, which are described in European Patents 488,248A1, 491,197A1 and 545,300, hereby incorporated by reference.

A preferred pyrrolotriazole coupler for use in the present invention is represented by the following structure (VIII):



wherein R<sup>10</sup> and R<sup>11</sup> each represents an alkyl group or an aryl group; R<sup>12</sup>, R<sup>13</sup> and R<sup>14</sup> each represents a hydrogen atom, an alkyl group or an aryl group; W represents a non-metallic atomic group necessary to form a saturated ring; R<sup>15</sup> represents a substituent; Y represents a coupling-off group as defined above, preferably a group X—CO—O—in which the acyl group is bonded to the pyrrolotriazole ring and X represents a heterocyclic group, a substituted amino group or an aryl group; and Z represents a hydrogen atom or a group capable of being released upon color development, as defined above.

In preferred compounds of formula (VIII), the alkyl group represented by R<sup>10</sup>, R<sup>11</sup>, R<sup>12</sup>, R<sup>13</sup> or R<sup>14</sup> is a straight chain, branched chain or cyclic alkyl group having from 1 to 36 carbon atoms, preferably a straight chain, branched chain or cyclic alkyl group having from 1 to 22 carbon atoms, and more preferably a straight chain or branched chain alkyl group having from 1 to 8 carbon atoms. Specific examples of the alkyl group include a methyl, ethyl, n-propyl, isopropyl, tert-butyl, tert-ethyl, tert-octyl, decyl, dodecyl, cetyl, stearyl, cyclohexyl or 2-ethylhexyl group.

The aryl group represented by R<sup>10</sup>, R<sup>11</sup>, R<sup>12</sup>, R<sup>13</sup> or R<sup>14</sup> in the Formula (VIII) is an aryl group having from 6 to 20 carbon atoms, preferably an aryl group having from 6 to 14 carbon atoms, and more preferably an aryl group having from 6 to 10 carbon atoms. Specific examples of the aryl group include a phenyl, 1-naphthyl, 2-naphthyl or 2-phenanthryl group.

The non-metallic atomic group necessary to form a saturated ring represented by W in the Formula (VIII) is a non-metallic atomic group necessary to form a 5-membered to 8-membered saturated ring which may be substituted. A non-metallic atom for forming the ring include a carbon atom, an oxygen atom, a nitrogen atom and a sulfur atom. The ring is preferably a 6-membered saturated carbon ring, and more preferably a cyclohexane ring substituted with an alkyl group having from 1 to 24 carbon atoms on the 4-position thereof.

The substituent represented by R<sup>15</sup> in the formula (VIII) includes, for example, a halogen atom (e.g., fluorine, chlorine, or bromine), an aliphatic group (preferably a straight chain or branched chain alkyl group having from 1 to 36 carbon atoms, an aralkyl group, an alkenyl group, an alkynyl group, a cycloalkyl group or a cycloalkenyl group, specifically, e.g., methyl, ethyl, propyl, isopropyl, tert-butyl, tridecyl, tert-ethyl, tert-octyl, 2-methanesulfonyl-ethyl, 3-(3-pentadecylphenoxy)propyl, 3-[4-[2-[4-(4-hydroxyphenylsulfonyl)phenoxy]dodecanamido]phenyl]propyl, 2-ethoxytridecyl, trifluoromethyl, cyclopentyl, or 3-(2,4-di-tert-amylphenoxy)propyl), an aryl group (preferably having from 6 to 36 carbon atoms, specifically, e.g., phenyl, 4-tert-butylphenyl, 2,4-di-tert-amylphenyl, 4-tetradecanamidophenyl, or 2-methoxyphenyl), a heterocyclic group (preferably having from 1 to 36 carbon atoms, specifically, e.g., 2-furyl, 2-thienyl, 2-pyrimidinyl, or 2-benzothiazolyl), a cyano group, a hydroxy group, a nitro group, a carboxy group, an amino group, an alkoxy group (preferably a straight chain, branched chain or cyclic alkoxy group having from 1 to 36 carbon atoms, specifically, e.g., methoxy, ethoxy, butoxy, 2-methoxyethoxy, 2-dodecyloxyethoxy, or 2-methanesulfonylethoxy), an aryloxy group (preferably having from 6 to 36 carbon atoms, specifically, e.g., phenoxy, 2-methylphenoxy, 4-tert-butylphenoxy, 3-nitrophenoxy, 3-tert-butylphenoxy, or 3-methoxycarbamoylphenoxy), an acylamino group (preferably having from 2 to 36 carbon atoms, specifically, e.g., acetamido, benzamido, tetradecanamido, 2-(2,4-di-tert-amylphenoxy)butanamido, 4-(3-tert-butyl-4-hydroxyphenoxy)butanamido, or 2-[4-(4-hydroxyphenylsulfonyl)phenoxy]decanamido), an alkylamino group (preferably having from 1 to 36 carbon atoms, specifically, e.g., methylamino, butylamino, dodecyl amino, diethylamino, or methylbutyl amino), an aryl amino group (preferably having from 6 to 36 carbon atoms, specifically, e.g., phenylamino, 2-chloroanilino, 2-chloro-5-tetradecanamidoanilino, 2-chloro-5-dodecyloxycarbonylanilino, N-acetylanilino, or 2-chloro-5-[2-(3-tert-butyl-4-hydroxyphenoxy)dodecanamido]anilino), a ureido group (preferably having from 2 to 36 carbon atoms, specifically, e.g., phenylureido, methylureido, or N,N-dibutylureido), a sulfamoylamino group (preferably having from 1 to 36 carbon atoms, specifically, e.g., N,N-dipropylsulfamoylamino, or N-methyl-N-decylsulfamoylamino), an alkylthio group (preferably having from 1 to 36 carbon atoms, specifically, e.g., methylthio, octylthio, tetradecylthio, 2-phenoxyethylthio, 3-phenoxypropylthio, or 3-(4-tert-butylphenoxy)propylthio), an arylthio group (preferably having from 6 to 36 carbon atoms, specifically, e.g., phenylthio, 2-butoxy-5-tert-octylphenylthio, 3-pentadecylphenylthio, 2-carboxyphenylthio, or 4-tetradecanamidophenylthio), an alkoxy carbonylamino group (preferably having from 2 to 36 carbon atoms, specifically, e.g., methoxycarbonylamino, or tetradecyloxycarbonylamino), a sulfonamido group (preferably an alkyl- or aryl-sulfonamido group having from 1 to 36 carbon atoms, specifically, e.g., methanesulfonamido, butanesulfonamido, octanesulfonamido, hexadecanesulfonamido,

benzenesulfonamido, p-toluenesulfonamido, octadecanesulfonamido, or 2-methoxy-5-tert-butylbenzenesulfonamido), a carbamoyl group (preferably having from 1 to 36 carbon atoms, e.g., N-ethylcarbamoyl, N,N-dibutylcarbamoyl, N-(2-dodecyloxyethyl)carbamoyl, N-methyl-N-dodecylcarbamoyl, or N-[3-(2,4-di-tert-amylphenoxy)propyl]-3-carbamoyl), a sulfamoyl group (preferably having from 1 to 36 carbon atoms, specifically, e.g., N-ethylsulfamoyl, N,N-dipropylsulfamoyl, N-(2-dodecyloxyethyl)sulfamoyl, N-ethyl-N-dodecylsulfamoyl, or N,N-diethylsulfamoyl), a sulfonyl group (preferably an alkyl- or aryl-sulfonyl group having from 1 to 36 carbon atoms, specifically, e.g., methanesulfonyl, octanesulfonyl, benzenesulfonyl, or toluenesulfonyl), an alkoxy carbonyl group (preferably having from 2 to 36 carbon atoms, specifically, e.g., methoxycarbonyl, butoxycarbonyl, 15 dodecyloxy carbonyl, or octadecyloxy carbonyl), a heterocyclic oxy group (preferably having from 1 to 36 carbon atoms, specifically, e.g., 1-phenyltetrazol-5-oxy, or 2-tetrahydropyranoxy), an azo group (e.g., phenylazo, 4-methoxyphenylazo, 4-pivaloylaminophenylazo, or 2-hydroxy-4-propanoylphenylazo), an acyloxy group (preferably having from 2 to 36 carbon atoms, specifically, e.g., acetoxy), a carbamoyloxy group (preferably having from 1 to 36 carbon atoms, specifically, e.g., N-methylcarbamoyloxy, or N-phenylcarbamoyloxy), a silyloxy group (preferably having from 3 to 36 carbon atoms, specifically, e.g., trimethylsilyloxy, or 20 dibutylmethylsilyloxy), an aryloxycarbonylamino group (preferably having from 7 to 36 carbon atoms, specifically, e.g., phenoxy carbonylamino), an imido group (preferably having from 4 to 36 carbon atoms, specifically, e.g., N-succinimido, N-phthalimido, or 3-octadecenylsuccinimido), a heterocyclic thio group (preferably having from 1 to 36 carbon atoms specifically, e.g., 2-benzothiazolylthio, 2,4-di-phenoxy-1,3,5-triazol-6-thio, or 2-pyridylthio), a sulfinyl group (preferably having from 1 to 36 carbon atoms, specifically e.g., dodecanesulfinyl, 3-pentadecylphenylsulfinyl, or 3-phenoxypropylsulfinyl), an alkyl-, aryl- or heterocyclic oxycarbonyl group (e.g., methoxycarbonyl, butoxycarbonyl, 30 dodecyloxy carbonyl, phenoxy carbonyl, 2-pentadecyloxy carbonyl), an alkyl-, aryl- or heterocyclic carbonylamino group (e.g., methoxycarbonylamino, tetradecyloxy carbonylamino, phenoxy carbonylamino, or 2,4-di-tert-butylphenoxy carbonylamino), a sulfonamido group (e.g., methanesulfonamido, hexadecanesulfonamido, 35 benzenesulfonamido, p-toluenesulfonamido, octadecanesulfonamido, or 2-methoxy-5-tert-butylbenzenesulfonamido), a carbamoyl group (e.g., N-ethylcarbamoyl, N,N-dibutylcarbamoyl, N-(2-dodecyloxyethyl)carbamoyl, N-methyl-N-dodecylcarbamoyl, or N-[3-(2,4-di-tert-amylphenoxy)propyl]-3-carbamoyl), a sulfamoyl group (e.g., N-ethylsulfamoyl, N,N-dipropylsulfamoyl, N-(2-dodecyloxyethyl)sulfamoyl, N-ethyl-N-dodecylsulfamoyl, or N,N-diethylsulfamoyl), a phosphonyl group (e.g., 45 phenoxyphosphonyl, octyloxyphosphonyl, or phenylphosphonyl), an imido group (e.g., N-succinimido, hydantoinyl, N-phthalimido, or 3-octadecenylsuccinimido), an azolyl group (e.g., imidazolyl, pyrazolyl, 50 3-chloropyrazol-1-yl, or triazolyl), a sulfo group, and an unsubstituted amino group.

R<sup>15</sup> is preferably an alkyl group, an aryl group, a heterocyclic group, a cyano group, a nitro group, an acylamino group, an arylamino group, a ureido group, a sulfamoylamino group, an alkylthio group, an arylthio group, an alkoxy carbonylamino group, a sulfonamido group, a carbamoyl group, a sulfamoyl group, a sulfonyl group, an alkoxy carbonyl group, an aryloxycarbonyl group, a hetero-

cycloxy group, an acyloxy group, a carbamoyloxy group, an aryloxycarbonyl amino group, an imido group, a heterocyclic thio group, a sulfinyl group, a phosphonyl group, an acyl group, or an azolyl group.

More preferably, R<sup>15</sup> is an alkyl group or an aryl group. Still more preferably, R<sup>15</sup> is an aryl group substituted at least with an alkyl group on the p-position thereof.

As mentioned above, Y is preferably a group X—CO—O— in which X represents a heterocyclic group, a substituted amino group or an aryl group as described above. A heterocyclic ring for forming the heterocyclic group represented by X is preferably a 5-membered to 8-membered ring containing a nitrogen atom, an oxygen atom or a sulfur atom as a hetero atom and having from 1 to 36 carbon atoms. A 5-membered or 6-membered nitrogen-containing heterocyclic ring which is connected to the carbonyl group through the nitrogen atom is more preferred. Among others, the 6-membered nitrogen-containing heterocyclic ring connecting through the nitrogen atom is particularly preferred.

Specific examples of the heterocyclic ring include imidazole, pyrazole, triazole, a lactam compound, 25 piperidine, pyrrolidine, pyrrole, morpholine, pyrazolidine, thiazolidine and pyrazoline. Preferred rings are morpholine and piperidine, and morpholine is particularly preferred.

A substituent for the substituted amino group include an aliphatic group, an aryl group and a heterocyclic group. Suitable examples of the aliphatic group include those described for R<sup>15</sup> above. The aliphatic group may be substituted with a cyano group, an alkoxy group (e.g., methoxy), an alkoxy carbonyl group (e.g., ethoxycarbonyl), a chlorine atom, a hydroxy group or a carboxyl group. Of the substituted amino groups, a disubstituted amino group is more preferred than a monosubstituted amino group.

The aryl group has preferably from 6 to 36 carbon atoms. 40 A monocyclic aryl group is more preferred. Specific examples of the aryl group include a phenyl, 4-tert-butylphenyl, 2-methylphenyl, 2,4,6-trimethylphenyl, 2-methoxyphenyl, 4-methoxyphenyl, 2,6-dichlorophenyl, 2-chlorophenyl or 2,4-dichlorophenyl group.

The coupler represented by the formula (VIII) may be a dimer or more, in which R<sup>15</sup> contains a residue of the coupler represented by the formula (VIII), or may be a homopolymer or a copolymer, in which R<sup>15</sup> contains a polymer chain. Typical examples of the homopolymer or copolymer include homopolymers or copolymers formed from an addition-polymerizable ethylenically unsaturated compound having a residue of the coupler represented by the formula (VIII). Such homopolymers or copolymers may contain one or more infrared forming repeating units containing a residue of the coupler represented by the formula (VIII). The copolymers may contain one or more non-color forming ethylenic monomers which do not couple with an oxidation product of an aromatic primary amine developing agent, such as acrylates, methacrylates or maleates.

The above-described pyrrolotriazole compounds can be synthesized as disclosed in U.S. Pat. No. 6,220,925 B1, hereby incorporated by reference.

65 In one embodiment, a particularly preferred class of pyrrolotriazole couplers are 1H-pyrrolo-[1,2-b][1,2,4]triazole compounds represented by formula (IX):



(IX)

5

10

15

20

wherein R is an alkyl group; R<sup>a</sup>, R<sup>b</sup>, R<sup>c</sup>, R<sup>a'</sup>, R<sup>b'</sup>, and R<sup>c'</sup>, each are a hydrogen atom or an alkyl group; R<sup>a</sup> and R<sup>b</sup>, and R<sup>a'</sup> and R<sup>b'</sup> may bond together to form a ring, 25 respectively; R<sup>16</sup> is a hydrogen atom or an alkyl group as defined above, and X is heterocyclic group as defined above, a substituted amino group, or an aryl group. Such compounds, its synthetic intermediates, 30 and methods for producing such intermediates are disclosed in published application EP 0 857 726 A1 to Shimada et al., filed Jan. 13, 1998, hereby incorporated by reference.

In formula (IX), R<sup>a</sup>, R<sup>b</sup>, R<sup>c</sup>, R<sup>a'</sup>, R<sup>b'</sup>, and R<sup>c'</sup> which may 35 be the same or different, each represent a hydrogen atom, or a straight chain or branched chain alkyl group having 1 to 24 carbon atoms, or a cyclic alkyl group (preferably having 3 to 8 carbon atoms). R<sup>16</sup> represents a hydrogen atom, or a straight chain or branched chain alkyl group having 1 to 36 40 carbon atoms, or a cyclic alkyl group (preferably having 3 to 8 carbon atoms).

Specific examples of some pyrrolotriazole couplers useful 45 in the present invention for forming infrared imaging dyes are as follows:



C-1

50

55

60

65

14  
-continued

C-2



C-3



C-4



C-5

15

-continued



16

The latter compound, in reaction with Developer D-2 below, will yield the following infrared dye:

DYE-1



This IR dye has a  $\lambda_{max}$  at about 785 nm.

In addition to a hue-shifted cyan coupler for producing an infrared image, it is possible to provide hue-shifting developing agents in the other imaging layers, for example, to produce a cyan color from a magenta dye, as disclosed in commonly assigned, copending Ser. No. 09/930,939, hereby incorporated by reference.

It may be desirable to combine the above-described IR dye-forming system, in a photothermographic element, with hypo-shifted cyan and magenta couplers. However, typically, the resulting infrared dye may be sufficiently broad that there is some overlap with the cyan and magenta dye peaks formed from conventional cyan and magenta couplers. Improved separation between the infrared-dye forming channel and the cyan- and magenta-dye forming channels can be achieved by using hypsochromically shifted cyan- and magenta couplers. In one embodiment, therefore, it may be desirable to employ a coupler with a lambda max between 550 and 650 in the red channel, and a coupler with a lambda max between 450 and 550 in the green channel. Improved separation between the cyan-dye forming channel and the infrared-dye forming channel can be achieved by using the cyan couplers disclosed in commonly assigned copending Ser. No. 09/930,939.

The specified dye-forming couplers useful in the invention can be incorporated in the imaging member in any manner known in the art. These methods include, but are not limited to, incorporation as oil-in-water emulsions, known colloquially in the photographic arts as "dispersions," as reverse phase emulsion, as solid particle dispersions, as multiphase dispersions, as molecular dispersions or "Fisher" dispersions, or as polymer loaded dispersions or loaded latex dispersions. When the multifunctional dye forming couplers are polymeric in nature, they can additionally be incorporated merely by physically diluting the polymeric coupler with vehicle. While the multifunctional dye forming coupler can be employed in the member at any concentration that enables the desired formation of a multicolor image, it is preferred that the multifunctional dye forming coupler be applied to the member at between about 50 and 3000 mg/m<sup>2</sup>. It is more preferred that the multifunctional dye forming coupler be applied to the member at between about 200 and 800 mg/m<sup>2</sup>.

The imaging member can further comprise an incorporated solvent. In one embodiment the multifunctional dye forming coupler is provided as an emulsion in such a solvent. In this embodiment, any of the high boiling organic solvents known in the photographic arts as "coupler solvents" can be employed. In this situation, the solvent acts as a manufacturing aid. Alternatively, the solvent can be incorporated separately. In both situations, the solvent can further function as a coupler stabilizer, a dye stabilizer, a reactivity enhancer or moderator or as a hue shifting agent, all as known in the photographic arts. Additionally, auxiliary solvents can be employed to aid dissolution of the multifunctional dye forming coupler in the coupler solvent. Particulars of coupler solvents and their use are described in the aforesaid mentioned references and at *Research Disclosure*, Item 37038 (1995), Section IX, Solvents, and Section XI, Surfactants, incorporated herein by reference. Some specific examples of coupler solvents include, but are not limited to, tritolyl phosphate, dibutyl phthalate, N,N-diethyldodecanamide, N,N-dibutyldodecanamide, tris(2-ethylhexyl)phosphate, acetyl tributyl citrate, 2,4-di-tert-pentylphenol, 2-(2-butoxyethoxy)ethyl acetate and 1,4-cyclohexyldimethylene bis(2-ethylhexanoate). The choice of coupler solvent and vehicle can influence the hue of dyes formed as disclosed by Merkel et al at U.S. Pat. Nos. 4,808,502 and 4,973,535. Typically, it is found that materials with a hydrogen bond donating ability can shift dyes bathochromically while materials with a hydrogen bond accepting ability can shift dyes hypsochromically. Additionally, use of materials with low polarizability can of itself promote hypsochromic dye hue shifts as well as promote dye aggregation. It is recognized that coupler ballasts often enable dyes and dye-coupler mixtures to function as self-solvents with a concomitant shift in hue. The polarizability, and the hydrogen bond donating and accepting ability of various materials are described by Kamlet et al in *J. Org. Chem.*, 48, 2877-87 (1983), the disclosures of which are incorporated by reference.

Generally one or more developer precursors are employed in the practice of this invention and are incorporated in the imaging element during manufacture, one of which is the blocked developer according to the present invention. Preferably, at least two types of developers are used. The developer precursors can release any developers known in the art that are coupling developers and enable the formation of distinctly colored dyes from the same coupler. By distinctly colored is meant that the dyes formed differ in the wavelength of maximum adsorption by at least 50 nm. It is preferred that these dyes differ in the maximum adsorption wavelength by at least 65 nm and more preferred that they differ in the maximum adsorption wavelength by at least 80 nm. It is further preferred that, in addition to the infrared dye, a magenta and a cyan dye are formed. In yet another embodiment multiple cyan dye forming, magenta dye forming or cyan dye forming developers can be individually employed to form a greater gamut of colors or to form colors at greater bit depth.

A cyan dye is a dye having a maximum absorption at between 580 and 700 nm, with preferably a maximum absorption between 590 and 680 nm, more preferably a peak absorption between 600 and 690 nm and most preferably a peak absorption between 605 and 680 nm. A magenta dye is a dye having a maximum absorption at between 500 and 580 nm, with preferably a maximum absorption between 515 and 565 nm, more preferably a peak absorption between 520 and 560 nm and most preferably a peak absorption between 525 and 555 nm. A yellow dye is a dye having a maximum

absorption at between 400 and 500 nm, with preferably a maximum absorption between 410 and 480 nm, more preferably a peak absorption between 435 and 465 nm and most preferably a peak absorption between 445 and 455 nm.

The concentrations and amounts of the developers and the dye-forming couplers according to the present invention will typically be chosen so as to enable the formation of dyes having a density at maximum absorption of at least 0.7, preferably a density of at least 1.0, more preferably a density of at least 1.3 and most preferably a density of at least 1.6. Further, the dyes will typically have a half height band width (HHWB) of between 70 and 170 nm in the region between 400 and 700 nm. Preferably, the HHWB will be less than 150 nm, more preferably less than 130 nm and most preferably less than 115 nm.

The photographic elements may further contain other image-modifying compounds such as "Development Inhibitor-Releasing" compounds (DIR's). Useful additional DIR's for elements of the present invention, are known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

A typical color negative film construction useful in the practice of the invention is illustrated by the following element, SCN-1:

| Element SCN-1 |                            |
|---------------|----------------------------|
| SOC           | Surface Overcoat           |
| BU            | Blue Recording Layer Unit  |
| IL1           | First Interlayer           |
| GU            | Green Recording Layer Unit |
| IL2           | Second Interlayer          |
| RU            | Red Recording Layer Unit   |
| AHU           | Antihalation Layer Unit    |
| S             | Support                    |
| SOC           | Surface Overcoat           |

Details of support construction are well understood in the art. Examples of useful supports are poly(vinylacetal) film, polystyrene film, poly(ethyleneterephthalate) film, poly(ethylene naphthalate) film, polycarbonate film, and related films and resinous materials, as well as paper, cloth, glass, metal, and other supports that withstand the anticipated processing conditions. The element can contain additional layers, such as filter layers, interlayers, overcoat layers, subbing layers, antihalation layers and the like. Transparent and reflective support constructions, including subbing layers to enhance adhesion, are disclosed in Section XV of *Research Disclosure*, September 1996, Number 389, Item 38957 (hereafter referred to as ("Research Disclosure I").

The photographic elements of the invention may also usefully include a magnetic recording material as described in *Research Disclosure*, Item 34390, November 1992, or a

transparent magnetic recording layer such as a layer containing magnetic particles on the underside of a transparent support as in U.S. Pat. No. 4,279,945, and U.S. Pat. No. 4,302,523.

Each of blue, green and red recording layer units BU, GU and RU are formed of one or more hydrophilic colloid layers and contain at least one radiation-sensitive silver halide emulsion. It is preferred that the green, and red recording units are subdivided into at least two recording layer sub-units to provide increased recording latitude and reduced image granularity. In the simplest contemplated construction each of the layer units or layer sub-units consists of a single hydrophilic colloid layer containing emulsion and coupler. When coupler present in a layer unit or layer sub-unit is coated in a hydrophilic colloid layer other than an emulsion containing layer, the coupler containing hydrophilic colloid layer is positioned to receive oxidized color developing agent from the emulsion during development. In this case, the coupler containing layer is usually the next adjacent hydrophilic colloid layer to the emulsion containing layer.

In order to ensure excellent image sharpness, and to facilitate manufacture and use in cameras, all of the sensitized layers are preferably positioned on a common face of the support. When in spool form, the element will be spooled such that when unspooled in a camera, exposing light strikes all of the sensitized layers before striking the face of the support carrying these layers. Further, to ensure excellent sharpness of images exposed onto the element, the total thickness of the layer units above the support should be controlled. Generally, the total thickness of the sensitized layers, interlayers and protective layers on the exposure face of the support are less than 35  $\mu\text{m}$ . In another embodiment, sensitized layers disposed on two sides of a support, as in a duplitzed film, can be employed.

In a preferred embodiment of this invention, the processed photographic film contains only limited amounts of color masking couplers, incorporated permanent  $D_{\min}$  adjusting dyes and incorporated permanent antihalation dyes. Generally, such films contain color masking couplers in total amount up to 0.6 mmol/ $\text{m}^2$ , preferably in amount up to about 0.2 mmol/ $\text{m}^2$ , more preferably in amounts up to about 0.05 mmol/ $\text{m}^2$ , and most preferably in amounts up to about 0.01 mmol/ $\text{m}^2$ .

The incorporated permanent  $D_{\min}$  adjusting dyes are generally present in total amounts up to about 0.2 mmol/ $\text{m}^2$ , preferably in amounts up to about 0.1 mmol/ $\text{m}^2$ , more preferably in amounts up to about 0.02 mmol/ $\text{m}^2$ , and most preferably in amounts up to about 0.005 mmol/ $\text{m}^2$ . The incorporated permanent antihalation density is up to about 0.6 in blue, green or red density, more preferably up to about 0.3 in blue, green or red density, even more preferably up to about 0.1 in blue, green or red density and most preferably up to about 0.05 in blue, green or red Status M density.

Limiting the amount of color masking couplers, permanent antihalation density and incorporated permanent  $D_{\min}$  adjusting dyes serves to reduce the optical density of the films, after processing, and thus improves the subsequent scanning and digitization of the imagewise exposed and processed films.

Overall, the limited  $D_{\min}$  and tone scale density enabled by controlling the quantity of incorporated color masking couplers, incorporated permanent  $D_{\min}$  adjusting dyes and antihalation and support optical density can serve to both limit scanning noise (which increases at high optical densities), and to improve the overall signal-to-noise characteristics of the film to be scanned. Relying on the digital correction step to provide color correction obviates the need for color masking couplers in the films.

Any convenient selection from among conventional radiation-sensitive silver halide emulsions can be incorporated within the layer units and used to provide the spectral absorptances of the invention. Most commonly high bromide emulsions containing a minor amount of iodide are employed. To realize higher rates of processing, high chloride emulsions can be employed. Radiation-sensitive silver chloride, silver bromide, silver iodobromide, silver iodochloride, silver chlorobromide, silver bromochloride, silver iodochlorobromide and silver iodobromochloride grains are all contemplated. The grains can be either regular or irregular (e.g., tabular). Tabular grain emulsions, those in which tabular grains account for at least 50 (preferably at least 70 and optimally at least 90) percent of total grain projected area are particularly advantageous for increasing speed in relation to granularity. To be considered tabular a grain requires two major parallel faces with a ratio of its equivalent circular diameter (ECD) to its thickness of at least 2. Specifically preferred tabular grain emulsions are those having a tabular grain average aspect ratio of at least 5 and, optimally, greater than 8. Preferred mean tabular grain thicknesses are less than 0.3  $\mu\text{m}$  (most preferably less than 0.2  $\mu\text{m}$ ). Ultrathin tabular grain emulsions, those with mean tabular grain thicknesses of less than 0.07  $\mu\text{m}$ , are specifically contemplated. However, in a preferred embodiment, a preponderance low reflectivity grains are preferred. By preponderance is meant that greater than 50% of the grain projected area is provided by low reflectivity silver halide grains. It is even more preferred that greater than 70% of the grain projected area be provided by low reflectivity silver halide grains. Low reflective silver halide grains are those having an average grain having a grain thickness >0.06, preferably >0.08, and more preferable >0.10 microns. The grains preferably form surface latent images so that they produce negative images when processed in a surface developer in color negative film forms of the invention.

Illustrations of conventional radiation-sensitive silver halide emulsions are provided by *Research Disclosure I*, cited above, I. Emulsion grains and their preparation. Chemical sensitization of the emulsions, which can take any conventional form, is illustrated in section IV. Chemical sensitization. Compounds useful as chemical sensitizers, include, for example, active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 4 to 8, and temperatures of from 30 to 80° C. Spectral sensitization and sensitizing dyes, which can take any conventional form, are illustrated by section V. Spectral sensitization and desensitization. The dye may be added to an emulsion of the silver halide grains and a hydrophilic colloid at any time prior to (e.g., during or after chemical sensitization) or simultaneous with the coating of the emulsion on a photographic element. The dyes may, for example, be added as a solution in water or an alcohol or as a dispersion of solid particles. The emulsion layers also typically include one or more antifoggants or stabilizers, which can take any conventional form, as illustrated by section VII. Antifoggants and stabilizers.

The silver halide grains to be used in the invention may be prepared according to methods known in the art, such as those described in *Research Disclosure I*, cited above, and James, *The Theory of the Photographic Process*. These include methods such as ammoniacal emulsion making, neutral or acidic emulsion making, and others known in the art. These methods generally involve mixing a water soluble silver salt with a water soluble halide salt in the presence of

a protective colloid, and controlling the temperature, pAg, pH values, etc, at suitable values during formation of the silver halide by precipitation.

In the course of grain precipitation one or more dopants (grain occlusions other than silver and halide) can be introduced to modify grain properties. For example, any of the various conventional dopants disclosed in *Research Disclosure I*, Section I. Emulsion grains and their preparation, sub-section G. Grain modifying conditions and adjustments, paragraphs (3), (4) and (5), can be present in the emulsions of the invention. In addition it is specifically contemplated to dope the grains with transition metal hexacoordination complexes containing one or more organic ligands, as taught by Olm, et al., U.S. Pat. No. 5,360,712, the disclosure of which is here incorporated by reference.

It is specifically contemplated to incorporate in the face centered cubic crystal lattice of the grains a dopant capable of increasing imaging speed by forming a shallow electron trap (hereinafter also referred to as a SET) as discussed in *Research Disclosure* Item 36736 published November 1994, here incorporated by reference.

The photographic elements of the present invention, as is typical, provide the silver halide in the form of an emulsion. Photographic emulsions generally include a vehicle for coating the emulsion as a layer of a photographic element. Useful vehicles include both naturally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), deionized gelatin, gelatin derivatives (e.g., acetylated gelatin, phthalated gelatin, and the like), and others as described in *Research Disclosure, I*. Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers. The vehicle can be present in the emulsion in any amount useful in photographic emulsions. The emulsion can also include any of the addenda known to be useful in photographic emulsions.

While any useful quantity of light sensitive silver, as silver halide, can be employed in the elements useful in this invention, it is preferred that the total quantity be not more than 4.5 g/m<sup>2</sup> of silver, preferably less. Silver quantities of less than 4.0 g/m<sup>2</sup> are preferred, and silver quantities of less than 3.5 g/m<sup>2</sup> are even more preferred. The lower quantities of silver improve the optics of the elements, thus enabling the production of sharper pictures using the elements. These lower quantities of silver are additionally important in that they enable rapid development and desilvering of the elements. Conversely, a silver coating coverage of at least 1.0 g of coated silver per m<sup>2</sup> of support surface area in the element is necessary to realize an exposure latitude of at least 2.7 log E while maintaining an adequately low graininess position for pictures intended to be enlarged. Silver coverages in excess of 1.5 g/m<sup>2</sup> are preferred while silver coverages in excess of 2.5 g/m<sup>2</sup> are more preferred.

It is common practice to coat one, two or three separate emulsion layers within a single dye image-forming layer unit. When two or more emulsion layers are coated in a single layer unit, they are typically chosen to differ in sensitivity. When a more sensitive emulsion is coated over a less sensitive emulsion, a higher speed is realized than when the two emulsions are blended. When a less sensitive

emulsion is coated over a more sensitive emulsion, a higher contrast is realized than when the two emulsions are blended. It is preferred that the most sensitive emulsion be located nearest the source of exposing radiation and the slowest emulsion be located nearest the support.

One or more of the layer units of the invention is preferably subdivided into at least two, and more preferably three or more sub-unit layers. It is preferred that all light sensitive silver halide emulsions in the color recording unit have spectral sensitivity in the same region of the visible spectrum. In this embodiment, while all silver halide emulsions incorporated in the unit have spectral absorptance according to invention, it is expected that there are minor differences in spectral absorptance properties between them.

15 In still more preferred embodiments, the sensitizations of the slower silver halide emulsions are specifically tailored to account for the light shielding effects of the faster silver halide emulsions of the layer unit that reside above them, in order to provide an imagewise uniform spectral response by the photographic recording material as exposure varies with low to high light levels. Thus higher proportions of peak light absorbing spectral sensitizing dyes may be desirable in the slower emulsions of the subdivided layer unit to account for on-peak shielding and broadening of the underlying layer 20 spectral sensitivity.

The interlayers IL1 and IL2 are hydrophilic colloid layers having as their primary function color contamination reduction-i.e., prevention of oxidized developing agent from migrating to an adjacent recording layer unit before reacting with dye-forming coupler. The interlayers are in part effective simply by increasing the diffusion path length that oxidized developing agent must travel. To increase the effectiveness of the interlayers to intercept oxidized developing agent, it is conventional practice to incorporate oxidized developer scavenging agents. Antistain agents (oxidized developing agent scavengers) can be selected from among those disclosed by *Research Disclosure I*, X. Dye image formers and modifiers, D. Hue modifiers/stabilization, paragraph (2). When one or more silver halide 30 emulsions in GU and RU are high bromide emulsions and, hence have significant native sensitivity to blue light, it is preferred to incorporate a yellow filter, such as Carey Lea silver or a yellow processing solution decolorizable dye, or a yellow thermally decolorizable dye, in IL1. Suitable yellow filter dyes can be selected from among those illustrated by *Research Disclosure I*, Section VIII. Absorbing and scattering materials, B. Absorbing materials. In elements of the instant invention, magenta colored filter materials are 35 absent from IL2 and RU.

40 50 The antihalation layer unit AHU typically contains a processing solution removable or decolorizable light absorbing material, or a thermally decolorizable dye, such as one or a combination of pigments and dyes. Suitable materials can be selected from among those disclosed in *Research Disclosure I*, Section VIII. Absorbing materials. A common alternative location for AHU is between the support S and the recording layer unit coated nearest the support.

55 The surface overcoats SOC are hydrophilic colloid layers that are provided for physical protection of the color negative elements during handling and processing. Each SOC 60 also provides a convenient location for incorporation of addenda that are most effective at or near the surface of the color negative element. In some instances the surface overcoat is divided into a surface layer and an interlayer, the latter functioning as spacer between the addenda in the surface layer and the adjacent recording layer unit. In another common variant form, addenda are distributed 65

between the surface layer and the interlayer, with the latter containing addenda that are compatible with the adjacent recording layer unit. Most typically the SOC contains addenda, such as coating aids, plasticizers and lubricants, antistats and matting agents, such as illustrated by *Research Disclosure I*, Section IX. Coating physical property modifying addenda. The SOC overlying the emulsion layers additionally preferably contains an ultraviolet absorber, such as illustrated by *Research Disclosure I*, Section VI. UV dyes/optical brighteners/luminescent dyes, paragraph (1).

Instead of the layer unit sequence of element SCN-1, alternative layer units sequences can be employed and are particularly attractive for some emulsion choices. Using high chloride emulsions and/or thin (<0.2  $\mu\text{m}$  mean grain thickness) tabular grain emulsions all possible interchanges of the positions of BU, GU and RU can be undertaken without risk of blue light contamination of the minus blue records, since these emulsions exhibit negligible native sensitivity in the visible spectrum. For the same reason, it is unnecessary to incorporate blue light absorbers in the inter-layers.

When the emulsion layers within a dye image-forming layer unit differ in speed, it is conventional practice to limit the incorporation of dye image-forming coupler in the layer of highest speed to less than a stoichiometric amount, based on silver. The function of the highest speed emulsion layer is to create the portion of the characteristic curve just above the minimum density-i.e., in an exposure region that is below the threshold sensitivity of the remaining emulsion layer or layers in the layer unit. In this way, adding the increased granularity of the highest sensitivity speed emulsion layer to the dye image record produced is minimized without sacrificing imaging speed.

The invention can be suitably applied to conventional color negative construction as illustrated. Color reversal film construction would take a similar form, with the exception that colored masking couplers would be completely absent; in typical forms, development inhibitor releasing couplers would also be absent. In preferred embodiments, the color negative elements are intended exclusively for scanning to produce three separate electronic color records. It is desirable that the dye image produced in each of the layer units be differentiable from that produced by each of the remaining layer units. To provide this capability of differentiation it is contemplated that each of the layer units contain one or more dye image-forming couplers chosen to produce image dye having an absorption half-peak bandwidth lying in a different spectral region. It is immaterial whether the blue, green or red recording layer unit forms a yellow, magenta or cyan dye having an absorption half peak bandwidth in the blue, green or red region of the spectrum, as is conventional in a color negative element intended for use in printing, or an absorption half-peak bandwidth in any other convenient region of the spectrum, ranging from the near ultraviolet (300–400 nm) through the visible and through the near infrared (700–1200 nm), so long as the absorption half-peak bandwidths of the image dye in the layer units extend over substantially non-coextensive wavelength ranges. The term “substantially non-coextensive wavelength ranges” means that each image dye exhibits an absorption half-peak band width that extends over at least a 25 (preferably 50) nm spectral region that is not occupied by an absorption half-peak band width of another image dye. Ideally the image dyes exhibit absorption half-peak band widths that are mutually exclusive.

When a layer unit contains two or more emulsion layers differing in speed, it is possible to lower image granularity

in the image to be viewed, recreated from an electronic record, by forming in each emulsion layer of the layer unit a dye image which exhibits an absorption half-peak band width that lies in a different spectral region than the dye images of the other emulsion layers of layer unit. This technique is particularly well suited to elements in which the layer units are divided into sub-units that differ in speed. This allows multiple electronic records to be created for each layer unit, corresponding to the differing dye images formed by the emulsion layers of the same spectral sensitivity. The digital record formed by scanning the dye image formed by an emulsion layer of the highest speed is used to recreate the portion of the dye image to be viewed lying just above minimum density. At higher exposure levels second and, optionally, third electronic records can be formed by scanning spectrally differentiated dye images formed by the remaining emulsion layer or layers. These digital records contain less noise (lower granularity) and can be used in recreating the image to be viewed over exposure ranges above the threshold exposure level of the slower emulsion layers. This technique for lowering granularity is disclosed in greater detail by Sutton U.S. Pat. No. 5,314,794, the disclosure of which is here incorporated by reference.

Each layer unit of the color negative elements of the invention produces a dye image characteristic curve gamma of less than 1.5, which facilitates obtaining an exposure latitude of at least 2.7 log E. A minimum acceptable exposure latitude of a multicolor photographic element is that which allows accurately recording the most extreme whites (e.g., a bride's wedding gown) and the most extreme blacks (e.g., a bride groom's tuxedo) that are likely to arise in photographic use. An exposure latitude of 2.6 log E can just accommodate the typical bride and groom wedding scene. An exposure latitude of at least 3.0 log E is preferred, since this allows for a comfortable margin of error in exposure level selection by a photographer. Even larger exposure latitudes are specifically preferred, since the ability to obtain accurate image reproduction with larger exposure errors is realized. Whereas in color negative elements intended for printing, the visual attractiveness of the printed scene is often lost when gamma is exceptionally low, when color negative elements are scanned to create digital dye image records, contrast can be increased by adjustment of the electronic signal information. When the elements of the invention are scanned using a reflected beam, the beam travels through the layer units twice. This effectively doubles gamma ( $\Delta D + \Delta A \log E$ ) by doubling changes in density ( $\Delta D$ ). Thus, gamma's as low as 1.0 or even 0.6 are contemplated and exposure latitudes of up to about 5.0 log E or higher are feasible. Gammas above 0.25 are preferred and gammas above 0.30 are more preferred. Gammas of between about 0.4 and 0.5 are especially preferred.

In a preferred embodiment the dye image is formed by the use of an incorporated developing agent, in reactive association with each color layer. More preferably, the incorporated developing agent is a blocked developing agent.

Examples of blocking groups that can be used in photographic elements of the present invention include, but are not limited to, the blocking groups described in U.S. Pat. No. 3,342,599, to Reeves; *Research Disclosure* (129 (1975) pp. 27–30) published by Kenneth Mason Publications, Ltd., Dudley Annex, 12a North Street, Emsworth, Hampshire PO10 7DQ, ENGLAND; U.S. Pat. No. 4,157,915, to Hamaoka et al.; U.S. Pat. No. 4,060,418, to Waxman and Mourning; and in U.S. Pat. No. 5,019,492. Other examples of blocking groups that can be used in photographic elements of the present invention include, but are not limited to,

25

the blocking groups described in U.S. Pat. No. 3,342,599, to Reeves; *Research Disclosure* (129 (1975) pp. 27-30) published by Kenneth Mason Publications, Ltd., Dudley Annex, 12a North Street, Emsworth, Hampshire PO10 7DQ, ENGLAND; U.S. Pat. No. 4,157,915, to Hamaoka et al.; U.S. Pat. No. 4,060,418, to Waxman and Mourning; and in U.S. Pat. No. 5,019,492. Particularly useful are those blocking groups described in U.S. application Ser. No. 09/476,234, filed Dec. 30, 1999, IMAGING ELEMENT CONTAINING A BLOCKED PHOTOGRAPHICALLY USEFUL COMPOUND; U.S. application Ser. No. 09/475,691, filed Dec. 30, 1999, IMAGING ELEMENT CONTAINING A BLOCKED PHOTOGRAPHICALLY USEFUL COMPOUND; U.S. application Ser. No. 09/475,703, filed Dec. 30, 1999, IMAGING ELEMENT CONTAINING A BLOCKED PHOTOGRAPHICALLY USEFUL COMPOUND; U.S. application Ser. No. 09/475,690, filed Dec. 30, 1999, IMAGING ELEMENT CONTAINING A BLOCKED PHOTOGRAPHICALLY USEFUL COMPOUND; and U.S. application Ser. No. 09/476,233, filed Dec. 30, 1999, PHOTOGRAPHIC OR PHOTOTHERMOPHOTOGRAPHIC ELEMENT CONTAINING A BLOCKED PHOTOGRAPHICALLY USEFUL COMPOUND. In one embodiment of the invention, the blocked developer may be represented by the following Structure I:



wherein,

DEV is a silver-halide color developing agent according to the present invention;

LINK 1 and LINK 2 are linking groups;

TIME is a timing group;

1 is 0 or 1;

m is 0, 1, or 2;

n is 0 or 1;

1+n is 1 or 2;

B is a blocking group or B is:



wherein B' also blocks a second developing agent DEV.

In a preferred embodiment of the invention, LINK 1 or LINK 2 are of structure II:



X represents carbon or sulfur;

Y represents oxygen, sulfur of N-R<sub>1</sub>, where R<sub>1</sub> is substituted or unsubstituted alkyl or substituted or unsubstituted aryl;

p is 1 or 2;

Z represents carbon, oxygen or sulfur;

r is 0 or 1;

with the proviso that when X is carbon, both p and r are 1, when X is sulfur, Y is oxygen, p is 2 and r is 0;

# denotes the bond to PUG (for LINK 1) or TIME (for LINK 2);

\\$ denotes the bond to TIME (for LINK 1) or T<sub>(t)</sub> substituted carbon (for LINK 2).

26

Illustrative linking groups include, for example,



TIME is a timing group. Such groups are well-known in the art such as (1) groups utilizing an aromatic nucleophilic substitution reaction as disclosed in U.S. Pat. No. 5,262,291; (2) groups utilizing the cleavage reaction of a hemiacetal (U.S. Pat. No. 4,146,396, Japanese Applications 60-249148; 60-249149); (3) groups utilizing an electron transfer reaction along a conjugated system (U.S. Pat. Nos. 4,409,323; 4,421,845; Japanese Applications 57-188035; 58-98728; 58-209736; 58-209738); and (4) groups using an intramolecular nucleophilic substitution reaction (U.S. Pat. No. 4,248,962).

Illustrative timing groups are illustrated by formulae T-1 through T-4.



T-1

wherein:

Nu is a nucleophilic group;

E is an electrophilic group comprising one or more carbon- or hetero-aromatic rings, containing an electron deficient carbon atom;

LINK 3 is a linking group that provides 1 to 5 atoms in the direct path between the nucleophilic site of Nu and the electron deficient carbon atom in E; and

a is 0 or 1.

Such timing groups include, for example:



These timing groups are described more fully in U.S. Pat. No. 5,262,291, incorporated herein by reference.



wherein

V represents an oxygen atom, a sulfur atom, or an



$R_{13}$  and  $R_{14}$  each represents a hydrogen atom or a substituent group;

$R_{15}$  represents a substituent group, and b represents 1 or 2

Typical examples of  $R_{13}$  and  $R_{14}$ , when they represent substituent groups, and  $R_{15}$  include



where,  $R_{16}$  represents an aliphatic or aromatic hydrocarbon residue, or a heterocyclic group; and  $R_{17}$  represents a hydrogen atom, an aliphatic or aromatic hydrocarbon residue, or a heterocyclic group,  $R_{13}$ ,  $R_{14}$  and  $R_{15}$  each may represent a divalent group, and any two of them combine with each other to complete a ring structure. Specific examples of the group represented by formula (T-2) are illustrated below.



wherein Nu 1 represents a nucleophilic group, and an oxygen or sulfur atom can be given as an example of

nucleophilic species; E1 represents an electrophilic group being a group which is subjected to nucleophilic attack by Nu 1; and LINK 4 represents a linking group which enables Nu 1 and E1 to have a steric arrangement such that an intramolecular nucleophilic substitution reaction can occur. Specific examples of the group represented by formula (T-3) are illustrated below.



wherein V,  $R_{13}$ ,  $R_{14}$  and b all have the same meaning as in formula (T-2), respectively. In addition,  $R_{13}$  and  $R_{14}$  may be joined together to form a benzene ring or a heterocyclic ring, or V may be joined with  $R_{13}$  or  $R_{14}$  to form a benzene or heterocyclic ring.  $Z_1$  and  $Z_2$  each independently represents a carbon atom or a nitrogen atom, and x and y each represents 0 or 1.

Specific examples of the timing group (T-4) are illustrated below.





Although the present invention is not limited to any type of developing agent or blocked developing agent, the following are merely some examples of photographically useful blocked developers that may be used in the invention to release developers for reaction with the pyrrolotriazole couplers for producing an infrared image in response to a selected hue of visible light. 50



D-2



D-3

D.4

D-5



D-1 55



60

65

**31**

-continued



D-7



D-8



D-9



D-10



D-11

**32**

-continued

D-12



D-13



D-14



D-15



D-16



65

A number of modifications of color negative elements have been suggested for accommodating scanning, as illustrated by *Research Disclosure I*, Section XIV. Scan facilitating features. These systems to the extent compatible with the color negative element constructions described above are contemplated for use in the practice of this invention.

It is also contemplated that the imaging element of this invention may be used with non-conventional sensitization schemes. For example, instead of using imaging layers sensitized to the red, green, and blue regions of the spectrum, the light-sensitive material may have one white-sensitive layer to record scene luminance, and two color-sensitive layers to record scene chrominance. Following development, the resulting image can be scanned and digitally reprocessed to reconstruct the full colors of the original scene as described in U.S. Pat. No. 5,962,205. The imaging element may also comprise a pan-sensitized emulsion with accompanying color-separation exposure. In this embodiment, the developers of the invention would give rise to a colored or neutral image that, in conjunction with the separation exposure, would enable full recovery of the original scene color values. In such an element, the image may be formed by either developed silver density, a combination of one or more conventional couplers, or "black" couplers such as resorcinol couplers. The separation exposure may be made either sequentially through appropriate filters, or simultaneously through a system of spatially discreet filter elements (commonly called a "color filter array").

The imaging element of the invention may also be a black and white image-forming material comprised, for example, of a pan-sensitized silver halide emulsion and a developer of the invention. In this embodiment, the image may be formed by developed silver density following processing, or by a coupler that generates a dye which can be used to carry the neutral image tone scale.

When the developed dyes are formed to read out the recorded scene exposures following chemical development of conventional exposed color photographic materials, the response of the red, green, and blue color recording units of the element can be accurately discerned by examining their densities. Densitometry is the measurement of transmitted light by a sample using selected colored filters to separate the imagewise response of the RGB image dye forming units into relatively independent channels. It is common to use Status M filters to gauge the response of color negative film elements intended for optical printing, and Status A filters for color reversal films intended for direct transmission viewing. In integral densitometry, the unwanted side and tail absorptions of the imperfect image dyes leads to a small amount of channel mixing, where part of the total response of, for example, a magenta channel may come from off-peak absorptions of either the yellow or cyan image dyes records, or both, in neutral characteristic curves. Such artifacts may be negligible in the measurement of a film's spectral sensitivity. By appropriate mathematical treatment of the integral density response, these unwanted off-peak density contributions can be completely corrected providing analytical densities, where the response of a given color record is independent of the spectral contributions of the other image dyes. Analytical density determination has been summarized in the *SPSE Handbook of Photographic Science and Engineering*, W. Thomas, editor, John Wiley and Sons, New York, 1973, Section 15.3, Color Densitometry, pp. 840-848.

Image noise can be reduced, where the images are obtained by scanning exposed and processed color negative film elements to obtain a manipulatable electronic record of

the image pattern, followed by reconversion of the adjusted electronic record to a viewable form. Image sharpness and colorfulness can be increased by designing layer gamma ratios to be within a narrow range while avoiding or minimizing other performance deficiencies, where the color record is placed in an electronic form prior to recreating a color image to be viewed. Whereas it is impossible to separate image noise from the remainder of the image information, either in printing or by manipulating an electronic image record, it is possible by adjusting an electronic image record that exhibits low noise, as is provided by color negative film elements with low gamma ratios, to improve overall curve shape and sharpness characteristics in a manner that is impossible to achieve by known printing techniques. Thus, images can be recreated from electronic image records derived from such color negative elements that are superior to those similarly derived from conventional color negative elements constructed to serve optical printing applications. The excellent imaging characteristics of the described element are obtained when the gamma ratio for each of the red, green and blue color recording units is less than 1.2. In a more preferred embodiment, the red, green, and blue light sensitive color forming units each exhibit gamma ratios of less than 1.15. In an even more preferred embodiment, the red and blue light sensitive color forming units each exhibit gamma ratios of less than 1.10. In a most preferred embodiment, the red, green, and blue light sensitive color forming units each exhibit gamma ratios of less than 1.10. In all cases, it is preferred that the individual color unit(s) exhibit gamma ratios of less than 1.15, more preferred that they exhibit gamma ratios of less than 1.10 and even more preferred that they exhibit gamma ratios of less than 1.05. In a like vein, it is preferred that the gamma ratios be greater than 0.8, more preferred that they be greater than 0.85 and most preferred that they be greater than 0.9. The gamma ratios of the layer units need not be equal. These low values of the gamma ratio are indicative of low levels of interlayer interaction, also known as interlayer interimage effects, between the layer units and are believed to account for the improved quality of the images after scanning and electronic manipulation. The apparently deleterious image characteristics that result from chemical interactions between the layer units need not be electronically suppressed during the image manipulation activity. The interactions are often difficult if not impossible to suppress properly using known electronic image manipulation schemes.

Elements having excellent light sensitivity are best employed in the practice of this invention. The elements should have a sensitivity of at least about ISO 50, preferably have a sensitivity of at least about ISO 100, and more preferably have a sensitivity of at least about ISO 200. Elements having a sensitivity of up to ISO 3200 or even higher are specifically contemplated. The speed, or sensitivity, of a color negative photographic element is inversely related to the exposure required to enable the attainment of a specified density above fog after processing. Photographic speed for a color negative element with a gamma of about 0.65 in each color record has been specifically defined by the American National Standards Institute (ANSI) as ANSI Standard Number PH 2.27-1981 (ISO (ASA Speed)) and relates specifically the average of exposure levels required to produce a density of 0.15 above the minimum density in each of the green light sensitive and least sensitive color recording unit of a color film. This definition conforms to the International Standards Organization (ISO) film speed rating. For the purposes of this

application, if the color unit gammas differ from 0.65, the ASA or ISO speed is to be calculated by linearly amplifying or deamplifying the gamma vs. log E (exposure) curve to a value of 0.65 before determining the speed in the otherwise defined manner.

The present invention also contemplates the use of photothermographic elements of the present invention in what are often referred to as single use cameras (or "film with lens" units). These cameras are sold with film preloaded in them and the entire camera is returned to a processor with the exposed film remaining inside the camera. The one-time-use cameras employed in this invention can be any of those known in the art. These cameras can provide specific features as known in the art such as shutter means, film winding means, film advance means, waterproof housings, single or multiple lenses, lens selection means, variable aperture, focus or focal length lenses, means for monitoring lighting conditions, means for adjusting shutter times or lens characteristics based on lighting conditions or user provided instructions, and means for camera recording use conditions directly on the film. These features include, but are not limited to: providing simplified mechanisms for manually or automatically advancing film and resetting shutters as described at Skarman, U.S. Pat. No. 4,226,517; providing apparatus for automatic exposure control as described at Matterson et al, U.S. Pat. No. 4,345,835; moisture-proofing as described at Fujimura et al, U.S. Pat. No. 4,766,451; providing internal and external film casings as described at Ohmura et al, U.S. Pat. No. 4,751,536; providing means for recording use conditions on the film as described at Taniguchi et al, U.S. Pat. No. 4,780,735; providing lens fitted cameras as described at Arai, U.S. Pat. No. 4,804,987; providing film supports with superior anti-curl properties as described at Sasaki et al, U.S. Pat. No. 4,827,298; providing a viewfinder as described at Ohmura et al, U.S. Pat. No. 4,812,863; providing a lens of defined focal length and lens speed as described at Ushiro et al, U.S. Pat. No. 4,812,866; providing multiple film containers as described at Nakayama et al, U.S. Pat. No. 4,831,398 and at Ohmura et al, U.S. Pat. No. 4,833,495; providing films with improved anti-friction characteristics as described at Shiba, U.S. Pat. No. 4,866,469; providing winding mechanisms, rotating spools, or resilient sleeves as described at Mochida, U.S. Pat. No. 4,884,087; providing a film patron or cartridge removable in an axial direction as described by Takei et al at U.S. Pat. Nos. 4,890,130 and 5,063,400; providing an electronic flash means as described at Ohmura et al, U.S. Pat. No. 4,896,178; providing an externally operable member for effecting exposure as described at Mochida et al, U.S. Pat. No. 4,954,857; providing film support with modified sprocket holes and means for advancing said film as described at Murakami, U.S. Pat. No. 5,049,908; providing internal mirrors as described at Hara, U.S. Pat. No. 5,084,719; and providing silver halide emulsions suitable for use on tightly wound spools as described at Yagi et al, European Patent Application 0,466,417 A.

While the film may be mounted in the one-time-use camera in any manner known in the art, it is especially preferred to mount the film in the one-time-use camera such that it is taken up on exposure by a thrust cartridge. Thrust cartridges are disclosed by Kataoka et al U.S. Pat. No. 5,226,613; by Zander U.S. Pat. No. 5,200,777; by Dowling et al U.S. Pat. No. 5,031,852; and by Robertson et al U.S. Pat. No. 4,834,306. Narrow bodied one-time-use cameras suitable for employing thrust cartridges in this way are described by Tobioka et al U.S. Pat. No. 5,692,221.

Cameras may contain a built-in processing capability, for example a heating element. Designs for such cameras

including their use in an image capture and display system are disclosed in Stoebe, et al., U.S. patent application Ser. No. 09/388,573 filed Sep. 1, 1999, incorporated herein by reference. The use of a one-time use camera as disclosed in said application is particularly preferred in the practice of this invention.

Photographic elements of the present invention are preferably imagewise exposed using any of the known techniques, including those described in *Research Disclosure I*, Section XVI. This typically involves exposure to light in the visible region of the spectrum, and typically such exposure is of a live image through a lens, although exposure can also be exposure to a stored image (such as a computer stored image) by means of light emitting devices (such as light emitting diodes, CRT and the like). The photothermographic elements are also exposed by means of various forms of energy, including ultraviolet and infrared regions of the electromagnetic spectrum as well as electron beam and beta radiation, gamma ray, x-ray, alpha particle, neutron radiation and other forms of corpuscular wave-like radiant energy in either non-coherent (random phase) or coherent (in phase) forms produced by lasers. Exposures are monochromatic, orthochromatic, or panchromatic depending upon the spectral sensitization of the photographic silver halide.

The elements as discussed above may serve as origination material for some or all of the following processes: image scanning to produce an electronic rendition of the capture image, and subsequent digital processing of that rendition to manipulate, store, transmit, output, or display electronically that image.

As mentioned above, the photographic elements of the present invention can be photothermographic elements of the type described in *Research Disclosure 17029* are included by reference. The photothermographic elements may be of type A or type B as disclosed in *Research Disclosure I*. Type A elements contain in reactive association a photosensitive silver halide, a reducing agent or developer, an activator, and a coating vehicle or binder. In these systems development occurs by reduction of silver ions in the photosensitive silver halide to metallic silver. Type B systems can contain all of the elements of a type A system in addition to a salt or complex of an organic compound with silver ion. In these systems, this organic complex is reduced during development to yield silver metal. The organic silver salt will be referred to as the silver donor. References describing such imaging elements include, for example, U.S. Pat. Nos. 3,457,075; 4,459,350; 4,264,725 and 4,741,992.

A photothermographic element comprises a photosensitive component that consists essentially of photographic silver halide. In the type B photothermographic material it is believed that the latent image silver from the silver halide acts as a catalyst for the described image-forming combination upon processing. In these systems, a preferred concentration of photographic silver halide is within the range of 0.01 to 100 moles of photographic silver halide per mole of silver donor in the photothermographic material.

The Type B photothermographic element comprises an oxidation-reduction image forming combination that contains an organic silver salt oxidizing agent. The organic silver salt is a silver salt which is comparatively stable to light, but aids in the formation of a silver image when heated to 80° C. or higher in the presence of an exposed photocatalyst (i.e., the photosensitive silver halide) and a reducing agent.

Suitable organic silver salts include silver salts of organic compounds having a carboxyl group. Preferred examples

thereof include a silver salt of an aliphatic carboxylic acid and a silver salt of an aromatic carboxylic acid. Preferred examples of the silver salts of aliphatic carboxylic acids include silver behenate, silver stearate, silver oleate, silver laureate, silver caprate, silver myristate, silver palmitate, silver maleate, silver fumarate, silver tartarate, silver furoate, silver linoleate, silver butyrate and silver camphorate, mixtures thereof, etc. Silver salts which are substitutable with a halogen atom or a hydroxyl group can also be effectively used. Preferred examples of the silver salts of aromatic carboxylic acid and other carboxyl group-containing compounds include silver benzoate, a silver-substituted benzoate such as silver 3,5-dihydroxybenzoate, silver o-methylbenzoate, silver m-methylbenzoate, silver p-methylbenzoate, silver 2,4-dichlorobenzoate, silver acetamidobenzoate, silver p-phenylbenzoate, etc., silver gallate, silver tannate, silver phthalate, silver terephthalate, silver salicylate, silver phenylacetate, silver pyromellitate, a silver salt of 3-carboxymethyl-4-methyl-4-thiazoline-2-thione or the like as described in U.S. Pat. No. 3,785,830, and silver salt of an aliphatic carboxylic acid containing a thioether group as described in U.S. Pat. No. 3,330,663.

Furthermore, a silver salt of a compound containing an imino group can be used. Preferred examples of these compounds include a silver salt of benzotriazole and a derivative thereof as described in Japanese patent publications 30270/69 and 18146/70, for example a silver salt of benzotriazole or methylbenzotriazole, etc., a silver salt of a halogen substituted benzotriazole, such as a silver salt of 5-chlorobenzotriazole, etc., a silver salt of 1,2,4-triazole, a silver salt of 3-amino-5-mercaptopbenzyl-1,2,4-triazole, of 1H-tetrazole as described in U.S. Pat. No. 4,220,709, a silver salt of imidazole and an imidazole derivative, and the like.

A second silver salt with a fog inhibiting property may also be used. The second silver organic salt, or thermal fog inhibitor, according to the present invention include silver salts of thiol or thione substituted compounds having a heterocyclic nucleus containing 5 or 6 ring atoms, at least one of which is nitrogen, with other ring atoms including carbon and up to two hetero-atoms selected from among oxygen, sulfur and nitrogen are specifically contemplated. Typical preferred heterocyclic nuclei include triazole, oxazole, thiazole, thiazoline, imidazoline, imidazole, diazole, pyridine and triazine. Preferred examples of these heterocyclic compounds include a silver salt of 2-mercaptopbenzimidazole, a silver salt of 2-mercapto-5-aminothiadiazole, a silver salt of 5-carboxylic-1-methyl-2-phenyl-4-thiopyridine, a silver salt of mercaptotriazine, a silver salt of 2-mercaptopbenzoxazole.

The second organic silver salt may be a derivative of a thionamide. Specific examples would include but not be limited to the silver salts of 6-chloro-2-mercaptopbenzothiazole, 2-mercaptop-thiazole, naphtho(1,2-d)thiazole-2 (1H)-thione, 4-methyl-4-thiazoline-2-thione, 2-thiazolidinethione, 4,5-dimethyl-4-thiazoline-2-thione, 4-methyl-5-carboxy-4-thiazoline-2-thione, and 3-(2-carboxyethyl)-4-methyl-4-thiazoline-2-thione.

Preferably, the second organic silver salt is a derivative of a mercapto-triazole. Specific examples would include, but not be limited to, a silver salt of 3-mercaptop-4-phenyl-1,2,4-triazole and a silver salt of 3-mercaptop-1,2,4-triazole.

Most preferably the second organic salt is a derivative of a mercapto-tetrazole. In one preferred embodiment, a mer-

capto tetrazole compound useful in the present invention is represented by the following structure:

MF-1



10 wherein n is 0 or 1, and R is independently selected from the group consisting of substituted or unsubstituted alkyl, aralkyl, or aryl. Substituents include, but are not limited to, C1 to C6 alkyl, nitro, halogen, and the like, which substituents do not adversely affect the thermal fog inhibiting effect of the silver salt. Preferably, n is 1 and R is an alkyl having 1 to 6 carbon atoms or a substituted or unsubstituted phenyl group. Specific examples include but are not limited to silver salts of 1-phenyl-5-mercaptop-tetrazole, 1-(3-acetamido)-5-mercaptop-tetrazole, or 1-[3-(2-sulfo)benzamidophenyl]-5-mercaptop-tetrazole.

15 The photosensitive silver halide grains and the organic silver salt are coated so that they are in catalytic proximity during development. They can be coated in contiguous layers, but are preferably mixed prior to coating.

20 25 Conventional mixing techniques are illustrated by *Research Disclosure*, Item 17029, cited above, as well as U.S. Pat. No. 3,700,458 and published Japanese patent applications Nos. 32928/75, 13224/74, 17216/75 and 42729/76.

30 The photothermographic element can comprise a thermal solvent. Examples of useful thermal solvents. Examples of thermal solvents, for example, salicylanilide, phthalimide, N-hydroxyphthalimide, N-potassium-phthalimide, succinimide, N-hydroxy-1,8-naphthalimide, phthalazine, 1-(2H)-phthalazinone, 2-acetylphthalazinone, benzalanilide, and benzenesulfonamide. Prior-art thermal solvents are disclosed, for example, in U.S. Pat. No. 6,013,420 to Winderer. Examples of toning agents and toning agent combinations are described in, for example, *Research Disclosure*, June 1978, Item No. 17029 and U.S. Pat. No. 4,123,282.

35 40 45 Photothermographic elements as described can contain addenda that are known to aid in formation of a useful image. The photothermographic element can contain development modifiers that function as speed increasing compounds, sensitizing dyes, hardeners, anti-static agents, plasticizers and lubricants, coating aids, brighteners, absorbing and filter dyes, such as described in *Research Disclosure*, December 1978, Item No. 17643 and *Research Disclosure*, June 1978, Item No. 17029.

50 After imagewise exposure of a photothermographic element, the resulting latent image can be developed in a variety of ways. The simplest is by overall heating the element to thermal processing temperature. This overall heating merely involves heating the photothermographic element to a temperature within the range of about 90° C. to about 180° C. until a developed image is formed, such as within about 0.5 to about 60 seconds. By increasing or decreasing the thermal processing temperature a shorter or longer time of processing is useful. A preferred thermal processing temperature is within the range of about 100° C. to about 160° C. Heating means known in the photothermographic arts are useful for providing the desired processing temperature for the exposed photothermographic element. The heating means is, for example, a simple hot plate, iron, roller, heated drum, microwave heating means, heated air, vapor or the like.

It is contemplated that the design of the processor for the photothermographic element be linked to the design of the cassette or cartridge used for storage and use of the element. Further, data stored on the film, or cartridge may be used to modify processing conditions or scanning of the element. Methods for accomplishing these steps in the imaging system are disclosed by Stoebe, et al., U.S. Pat. No. 6,062,746 and Szajewski, et al., U.S. Pat. No. 6,048,110, commonly assigned, which are incorporated herein by reference. The use of an apparatus whereby the processor can be used to write information onto the element, information which can be used to adjust processing, scanning, and image display is also envisaged. This system is disclosed in now allowed Stoebe, et al., U.S. patent applications Ser. No. 09/206,914 filed Dec. 7, 1998 and Ser. No. 09/333,092 filed Jun. 15, 1999, which are incorporated herein by reference.

Thermal processing is preferably carried out under ambient conditions of pressure and humidity. Conditions outside of normal atmospheric pressure and humidity are useful.

The components of the photothermographic element can be in any location in the element that provides the desired image. If desired, one or more of the components can be in one or more layers of the element. For example, in some cases, it is desirable to include certain percentages of the reducing agent, toner, stabilizer and/or other addenda in the overcoat layer over the photothermographic image-recording layer of the element. This, in some cases, reduces migration of certain addenda in the layers of the element.

In the preferred embodiment of a photothermographic film according to the present invention, the processing time to first image (either hard or soft display for customer/consumer viewing), including (i) thermal development of a film, (ii) scanning, and (iii) the formation of the positive image from the developed film, is suitably less than 5 minutes, preferably less than 3.5 minutes, more preferably less than 2 minutes, most preferably less than about 1 minute.

In view of advances in the art of scanning technologies, it has now become natural and practical for photothermographic color films such as disclosed in EP 0762 201 to be scanned, which can be accomplished without the necessity of removing the silver or silver-halide from the negative, although special arrangements for such scanning can be made to improve its quality. See, for example, Simmons U.S. Pat. No. 5,391,443.

Algorithms to reduce image noise and improve sharpness in the red, green, and blue channels of scanned images are well known in the art. However, if an infrared coupler is used to carry visible scene information in a photothermographic film, the accompanying scan may have additional noise or sharpness loss due to the CCD capture characteristics at long wavelengths. Image-processing algorithms specifically designed for an infrared channel may be required. Furthermore, it may be advantageous to match scanner diodes to the IR dye absorption peak. The diodes used in area array scanners are typically matched to the dyes used in the media to be scanned. The use of an IR dye in a photothermographic film will require the presence of IR diodes, preferably matched to the absorption characteristics of the dye. In one embodiment, a photothermographic film element containing an infrared coupler and developer according to the present invention, in the same layer, is exposed, processed, and then scanned with an area array CCD scanner illuminated with a diode having a wavelength between 760 and 800 nm.

It may also be advantageous for the IR dye-forming layer to be furthest from scanner during scanning operation. An

infrared dye-forming layer will experience the least amount of scattering during a scanning operation. Therefore, it would be preferable to locate the IR dye-containing layer furthest from the scanner element during the scanning operation. In one embodiment, an IR dye-forming layer containing an infrared dye forming coupler and developer according to the present invention is coated in association with a blue-sensitized emulsion in the top-most imaging layer of a multilayer film. Following processing, the film is oriented during scanning so that it is illuminated from the top (emulsion-side), with the capture element located on the support side of the coating. In a second embodiment, the infrared dye-forming layer comprises an infrared dye forming coupler and developer in association with a red-sensitized silver halide emulsion in the bottom-most imaging layer of a color negative film. Following processing, the film is oriented during scanning so that it is illuminated from the bottom (support-side), with the capture element located on the emulsion (top) side of the coating.

The use of an infrared dye-forming coupler to record visible (R, G, or B) scene information in a photothermographic film can lead to decreased light scattering and improvements in film scanning properties. However, current color algorithms use conventional color mapping (B→B, G→G, R→R) techniques to reproduce scene colors. An IR imaging layer, therefore, would require a modified algorithm (such as, G→B, R→G, and IR→R), as will be understood by the skilled artisan. Thus, it may be desirable, when a photothermographic film element comprising at least one light-sensitive layer containing the infrared dye forming coupler according to the present invention is exposed, processed, and scanned with R, G, IR, for an image processing algorithm then re-maps the R, G, and IR densities to the appropriate R, G, B color space.

Following development and scanning (or at least a first scanning), it may be desirable to remove or stabilize the retained silver halide and organic silver salt in a film, in order to render the PTG film to an archival state. Furthermore, the silver coated in the PTG film (silver halide, silver donor, and metallic silver) is unnecessary to the dye image produced, and this silver is valuable and the desire is to recover it is high.

Thus, it may be desirable to remove, in subsequent processing steps, one or more of the silver containing components of the film: the silver halide, one or more silver donors, the silver-containing thermal fog inhibitor if present, and/or the silver metal. The three main sources are the developed metallic silver, the silver halide, and the silver donor. Alternately, it may be desirable to stabilize the silver halide in the photothermographic film. Silver can be wholly or partially stabilized/removed based on the total quantity of silver and/or the source of silver in the film.

The removal of the silver halide and silver donor can be accomplished with a common fixing chemical as known in the photographic arts. Specific examples of useful chemicals include: thioethers, thioureas, thiols, thiones, thionamides, amines, quaternary amine salts, ureas, thiosulfates, thiocyanates, bisulfites, amine oxides, iminodiethanol-sulfur dioxide addition complex, amphoteric amines, bisulfonylmethanes, and the carbocyclic and heterocyclic derivatives of these compounds. These chemicals have the ability to form a soluble complex with silver ion and transport the silver out of the film into a receiving vehicle. The receiving vehicle can be another coated layer (laminated) or a conventional liquid processing bath.

The stabilization of the silver halide and silver donor can also be accomplished with a common stabilization chemical.

The previously mentioned silver salt removal compounds can be employed in this regard. With stabilization, the silver is not necessarily removed from the film, although the fixing agent and stabilization agents could very well be a single chemical. The physical state of the stabilized silver is no longer in large (>50 nm) particles as it was for the silver halide and silver donor, so the stabilized state is also advantaged in that light scatter and overall density is lower, rendering the image more suitable for scanning.

The removal of the metallic silver is more difficult than removal of the silver halide and silver donor. In general, two reaction steps are involved. The first step is to bleach the metallic silver to silver ion. The second step may be identical to the removal/stabilization step(s) described for silver halide and silver donor above. Metallic silver is a stable state that does not compromise the archival stability of the PTG film. Therefore, if stabilization of the PTG film is favored over removal of silver, the bleach step can be skipped and the metallic silver left in the film. In cases where the metallic silver is removed, the bleach and fix steps can be done together (called a blix) or sequentially (bleach+fix).

The process could involve one or more of the scenarios or permutations of steps. The steps can be done one right after another or can be delayed with respect to time and location. For instance, heat development and scanning can be done in a remote kiosk, then bleaching and fixing accomplished several days later at a retail photofinishing lab. In one embodiment, multiple scanning of images is accomplished. For example, an initial scan may be done for soft display or a lower cost hard display of the image after heat processing, then a higher quality or a higher cost secondary scan after stabilization is accomplished for archiving and printing, optionally based on a selection from the initial display.

For illustrative purposes, a non-exhaustive list of photothermographic film processes involving a common dry heat development step are as follows:

1. heat development=>scan=>stabilize (for example, with a laminate)=>scan=>obtain returnable archival film.
2. heat development=>fix bath=>water wash=>dry=>scan=>obtain returnable archival film
3. heat development=>scan=>blix bath=>dry=>scan=>recycle all or part of the silver in film
4. heat development=>bleach laminate=>fix laminate=>scan=>(recycle all or part of the silver in film)
5. heat development=>scan=>blix bath=>wash=>fix bath=>wash=>dry=>obtain returnable archival film
6. heat development=>relatively rapid, low quality scan
7. heat development=>bleach=>wash=>fix=>wash=>dry=>relatively slow, high quality scan

Photothermographic or photographic elements of the present invention can also be subjected to low-volume processing ("substantially dry" or "apparently dry") which is defined as photographic processing where the volume of applied developer solution is between about 0.1 to about 10 times, preferably about 0.5 to about 10 times, the volume of solution required to swell the photographic element. This processing may take place by a combination of solution application, external layer lamination, and heating. It is specifically contemplated that any components described in the preceding sections that are not necessary for the formation or stability of latent image in the origination film element can be removed from the film element altogether and contacted at any time after exposure for the purpose of carrying out photographic processing, using the methods described below.

A low-volume photothermographic element may receive some or all of the following three treatments:

(I) Application of a solution directly to the film by any means, including spray, inkjet, coating, gravure process and the like.

(II) Soaking of the film in a reservoir containing a processing solution. This process may also take the form of dipping or passing an element through a small cartridge.

(III) Lamination of an auxiliary processing element to the imaging element. The laminate may have the purpose of providing processing chemistry, removing spent chemistry, or transferring image information from the latent image recording film element. The transferred image may result from a dye, dye precursor, or silver containing compound being transferred in a image-wise manner to the auxiliary processing element.

Heating of the element during processing may be effected by any convenient means, including a simple hot plate, iron, roller, heated drum, microwave heating means, heated air, vapor, or the like. Heating may be accomplished before, during, after, or throughout any of the preceding treatments I-III. Heating may cause processing temperatures ranging from room temperature to 100° C.

Once developed dye image records (or the like) have been formed in the processed photographic elements of the invention, conventional techniques can be employed for retrieving the image information for each color record and manipulating the record for subsequent creation of a color balanced viewable image. For example, it is possible to scan the photothermographic element successively within the appropriate regions of the spectrum or to incorporate appropriate light within a single scanning beam that is divided and passed through appropriate filters to form separate scanning

beams for each color record. A simple technique is to scan the photothermographic element point-by-point along a series of laterally offset parallel scan paths. The intensity of light passing through the element at a scanning point is noted by a sensor which converts radiation received into an electrical signal. Most generally this electronic signal is further manipulated to form a useful electronic record of the image. For example, the electrical signal can be passed through an analog-to-digital converter and sent to a digital computer together with location information required for pixel (point) location within the image. In another embodiment, this electronic signal is encoded with colorimetric or tonal information to form an electronic record that is suitable to allow reconstruction of the image into viewable forms such as computer monitor displayed images, television images, printed images, and so forth.

It is contemplated that many of imaging elements of this invention will be scanned prior to the removal of silver halide from the element. The remaining silver halide yields a turbid coating, and it is found that improved scanned image quality for such a system can be obtained by the use of scanners that employ diffuse illumination optics. Any technique known in the art for producing diffuse illumination can be used. Preferred systems include reflective systems, that employ a diffusing cavity whose interior walls are specifically designed to produce a high degree of diffuse reflection, and transmissive systems, where diffusion of a beam of specular light is accomplished by the use of an optical element placed in the beam that serves to scatter light. Such elements can be either glass or plastic that either incorporate a component that produces the desired scattering, or have been given a surface treatment to promote the desired scattering.

43

One of the challenges encountered in producing images from information extracted by scanning is that the number of pixels of information available for viewing is only a fraction of that available from a comparable classical photographic print. It is, therefore, even more important in scan imaging to maximize the quality of the image information available. Enhancing image sharpness and minimizing the impact of aberrant pixel signals (i.e., noise) are common approaches to enhancing image quality. A conventional technique for minimizing the impact of aberrant pixel signals is to adjust each pixel density reading to a weighted average value by factoring in readings from adjacent pixels, closer adjacent pixels being weighted more heavily.

The elements of the invention can have density calibration patches derived from one or more patch areas on a portion of unexposed photographic recording material that was subjected to reference exposures, as described by Wheeler et al U.S. Pat. No. 5,649,260, Koeng et al U.S. Pat. No. 5,563,717, and by Cosgrove et al U.S. Pat. No. 5,644,647.

Illustrative systems of scan signal manipulation, including techniques for maximizing the quality of image records, are disclosed by Bayer U.S. Pat. No. 4,553,156; Urabe et al U.S. Pat. No. 4,591,923; Sasaki et al U.S. Pat. No. 4,631,578; Alkofer U.S. Pat. No. 4,654,722; Yamada et al U.S. Pat. No. 4,670,793; Klees U.S. Pat. Nos. 4,694,342 and 4,962,542; Powell U.S. Pat. No. 4,805,031; Mayne et al U.S. Pat. No. 4,829,370; Abdulwahab U.S. Pat. No. 4,839,721; Matsunawa et al U.S. Pat. Nos. 4,841,361 and 4,937,662; Mizukoshi et al U.S. Pat. No. 4,891,713; Petilli U.S. Pat. No. 4,912,569; Sullivan et al U.S. Pat. Nos. 4,920,501 and 5,070,413; Kimoto et al U.S. Pat. No. 4,929,979; Hiroswa et al U.S. Pat. No. 4,972,256; Kaplan U.S. Pat. No. 4,977,521; Sakai U.S. Pat. No. 4,979,027; Ng U.S. Pat. No. 5,003,494; Katayama et al U.S. Pat. No. 5,008,950; Kimura et al U.S. Pat. No. 5,065,255; Osamu et al U.S. Pat. No. 5,051,842; Lee et al U.S. Pat. No. 5,012,333; Bowers et al U.S. Pat. No. 5,107,346; Telle U.S. Pat. No. 5,105,266; MacDonald et al U.S. Pat. No. 5,105,469; and Kwon et al U.S. Pat. No. 5,081,692. Techniques for color balance adjustments during scanning are disclosed by Moore et al U.S. Pat. No. 5,049,984 and Davis U.S. Pat. No. 5,541,645.

The digital color records once acquired are in most instances adjusted to produce a pleasingly color balanced image for viewing and to preserve the color fidelity of the image bearing signals through various transformations or renderings for outputting, either on a video monitor or when printed as a conventional color print. Preferred techniques for transforming image bearing signals after scanning are disclosed by Giorgianni et al U.S. Pat. No. 5,267,030, the disclosures of which are herein incorporated by reference. Further illustrations of the capability of those skilled in the art to manage color digital image information are provided by Giorgianni and Madden *Digital Color Management*, Addison-Wesley, 1998.

#### PREPARATIVE EXAMPLES

The following examples illustrate the synthesis of representative blocked compounds useful in the invention.

44

#### Preparation of D-2



#### Preparation of 2

Water (450 mL) was slowly added at 0° C. to a mixture of 2,6-dimethyl-4-(N,N-diethyl)aniline diotosylate (1) (268.4 g, 0.50 mol), potassium bicarbonate (500.6 g, 5.00 mol) and dichloromethane (900 mL), followed by a 1.9M toluene solution of phosgene (550 mL, 1.00 mol) at 4–7° C. over a period of 30 min. Following the addition, the mixture was stirred cold for 30 min and diluted with dichloromethane (750 mL) and water (1000 mL). The layers were separated and the aqueous one extracted with dichloromethane (350 mL). Combined organic solutions were dried over sodium sulfate and the solvents were distilled off in vacuo at 45° C. The crude product was dissolved in ligroin (700 mL), the solution treated with charcoal, filtered through SuperCel and concentrated in vacuo at 50° C., giving 111.0 g (0.50 mol, 100%) of isocyanate 2 as a yellow oil. <sup>1</sup>HNMR (CDCl<sub>3</sub>): δ 6.35 (s, 2H), 3.30 (q, 4H), 2.25 (s, 6H), 1.15 (t, 6H).

#### Preparation of D-2

A solution of isocyanate 2 (177.6 g, 0.81 mol), diol 3 (87.1 g, 0.375 mol) and dibutyltin diacetate (1 mL) in 900 mL of acetonitrile was stirred at 50° C. under nitrogen for 3 days. The mixture was cooled to room temperature, filtered and the filtrate taken to dryness. The crystalline residue was stirred with isopropyl ether (500 mL), the product collected by filtration, washed with isopropyl ether (2×250 mL) and then ethanol (2×250 mL). Yield 220.9 g (0.33 mol, 88%), m.p. 173–175° C.

#### Preparation of D-3, D-4 and D-9

Blocked developers D-3, D-4 and D-9 were prepared as described above for D-2 from isocyanate 2 and appropriate alcohols in the presence of catalytic amounts of dibutyltin diacetate. The yields and melting points are listed below in Table 1 below.

TABLE 1

| Developer | Yield (%) | m.p. (° C.) |
|-----------|-----------|-------------|
| D-3       |           | 161–163     |
| D-4       | 84        | 91–93       |
| D-9       | 79        | 110–114     |

## PHOTOGRAPHIC EXAMPLES

Photothermographic coating examples were prepared using the following components:

Developers D-17, D-2, or D-12: Developers were incorporated into the photographic coatings as ball-milled dispersions. The dispersions were prepared by ball-milling the compounds with zirconia beads in water. TRITON X-200 was added to the dispersions as a surfactant. Typically, the developers were incorporated into the slurry at 10% (w/w), and the TRITON X-200 was added at a level of 10% by weight of the developer.



Couplers C-9 and C-10: Couplers were incorporated into the photographic coatings as conventional dispersions using a high-boiling organic liquid as solvent. Coupler C-9 was dispersed with an equal weight of tricresyl phosphate in aqueous gelatin. The final weight percent of the coupler in the dispersion was 6%. The gelatin content of the dispersion was also 6%. Coupler C-10 was dispersed in the same manner.

Coupler C-9



Coupler C-10



Melt former MF-1: A dispersion of salicylanilide (MF-1) was media-milled to give a dispersion containing 30% salicylanilide, with 4% TRITON X-200 surfactant and 4% polyvinyl pyrrolidone added relative to the weight of salicylanilide. The dispersion was then diluted with water to provide a final salicylanilide concentration of 25%.

MF-1



Silver salt dispersion SS-1: A stirred reaction vessel was charged with 431 g of lime processed gelatin and 6569 g of distilled water. A solution containing 214 g of benzotriazole, 2150 g of distilled water, and 790 g of 2.5 molar sodium hydroxide was prepared (Solution B). The mixture in the reaction vessel was adjusted to a pAg of 7.25 and a pH of 8.00 by additions of Solution B, nitric acid, and sodium hydroxide as needed. A 41 solution of 0.54 molar silver nitrate was added to the kettle at 250 cc/minute, and the pAg

was maintained at 7.25 by a simultaneous addition of solution B. This process was continued until the silver nitrate solution was exhausted, at which point the mixture was concentrated by ultrafiltration. The resulting silver salt dispersion contained fine particles of silver benzotriazole. Silver salt dispersion SS-2: A stirred reaction vessel was charged with 431 g of lime processed gelatin and 6569 g of distilled water. A solution containing 320 g of 1-phenyl-5-mercaptopentetrazole, 2044 g of distilled water, and 790 g of 2.5 molar sodium hydroxide was prepared (Solution B). The mixture in the reaction vessel was adjusted to a pAg of 7.25 and a pH of 8.00 by additions of Solution B, nitric acid, and sodium hydroxide as needed. A 41 solution of 0.54 molar silver nitrate was added to the kettle at 250 cc/minute, and the pAg was maintained at 7.25 by a simultaneous addition of solution B. This process was continued until the silver nitrate solution was exhausted, at which point the mixture was concentrated by ultrafiltration. The resulting silver salt dispersion contained fine particles of the silver salt of 1-phenyl-5-mercaptopentetrazole.

Emulsion E-1: A silver halide tabular emulsion with a composition of 96% silver bromide and 4% silver iodide was prepared by conventional means. The resulting emulsion had an equivalent circular diameter of 1.2 microns and a thickness of 0.11 microns. This emulsion was spectrally sensitized to green light by addition of a combination of dyes SM-1 and SM-2 at a ratio of 4.5:1 and then chemical sensitized for optimum performance.



Emulsion E-2. A silver halide tabular emulsion with a composition of 97% silver bromide and 3% silver iodide was prepared by conventional means.



The resulting emulsion had an equivalent circular diameter of 0.6 microns and a thickness of 0.09 microns. This

emulsion was spectrally sensitized to blue light by addition of dye SY-1 dye and then chemically sensitized for optimum performance.

#### Example 1

Photothermographic coatings were prepared on 7 mil polyethylene-terephthalate (PET) support using the above-described components at the levels given in Table 1.

TABLE 1

|                                 |                |
|---------------------------------|----------------|
| Developer D-17 or D-2           | 1.34 mmol/sq m |
| Silver Salt SS-1                | 0.32 g Ag/sq m |
| Silver Salt SS-2                | 0.32 g Ag/sq m |
| Meltformer MF-1                 | 0.86 g/sq m    |
| Coupler C-9                     | 0.45 g/sq m    |
| Emulsion E-1 (green sensitized) | 0.86 g/sq m    |
| Gelatin Binder                  | 4.30 g/sq m    |

The coatings received an overcoat of 3.2 g/sq m gelatin, and were hardened with bis-vinylsulfonyl methane at 1.8% (w/w) of total gelatin. The coatings were exposed through a stepped exposure and subsequently processed by heating for 18 seconds at 161 degrees C. Following processing, the light-sensitive silver halide was removed from the coatings by fixing in a sodium thiosulfate bath. The spectrum of the coatings at Dmax was measured using a Perkin-Elmer Lambda20 UV/visible spectrophotometer. The coatings were scanned from 900 to 400 nm, and the results are given in Table 2.

TABLE 2

| Sample           | Coupler | Developer | Wavelength of maximum absorption (lambda max) |
|------------------|---------|-----------|-----------------------------------------------|
| 1-1 (Comparison) | C-9     | D-17      | 670 nm                                        |
| 1-2 (Invention)  | C-9     | D-2       | 785 nm                                        |

As seen in this example, the use of a pyrrolotriazole coupler with a hue-shifting developer leads to an excellent infrared dye with a lambda max of 785 nm.

#### Example 2

To demonstrate that not all couplers that generate a cyan dye with conventional developers generate good infrared dyes with a hue-shifting developer, additional photothermographic coatings were prepared using the components in Table 3. The coatings were prepared on 4 mil polyethylene-terephthalate support.

TABLE 3

|                                |                                                       |
|--------------------------------|-------------------------------------------------------|
| Developer D-17, D-2, or D-12   | 1.34 mmol/sq m (D-17 or D-2)<br>2.68 mmol/sq m (D-12) |
| Silver Salt SS-1               | 0.32 g Ag/sq m                                        |
| Silver Salt SS-2               | 0.32 g Ag/sq m                                        |
| Meltformer MF-1                | 0.86 g/sq m                                           |
| Coupler C-9 or C-10            | 0.70 mmol/sq m                                        |
| Emulsion E-2 (blue sensitized) | 0.86 g/sq m                                           |
| Gelatin Binder                 | 4.30 g/sq m                                           |

The coatings of example were exposed through a stepped exposure and subsequently processed by heating for 20 seconds at 155 degrees C. Following processing, the light-sensitive silver halide was removed from the coatings by fixing in a sodium thiosulfate bath. The spectrum of the coatings at Dmax was measured as before, and the results are presented in Table 4. In addition to the absorption maxima, the amount of bathochromic shift observed when a

conventional (CD-2 releasing) developer is replaced by a hue-shifting developer is also reported in Table 4 below.

TABLE 4

| Sample           | Coupler | Developer | Wavelength of Maximum Absorption (lambda max) | Bathochromic Shift |
|------------------|---------|-----------|-----------------------------------------------|--------------------|
| 2-1 (Comparison) | C-10    | D-17      | 696 nm                                        | —                  |
| 2-2 (Comparison) | C-10    | D-2       | 708 nm                                        | 12 nm              |
| 2-3 (Comparison) | C-10    | D-12      | 732 nm                                        | 36 nm              |
| 2-4 (Comparison) | C-9     | D-17      | 678 nm                                        | —                  |
| 2-5 (Invention)  | C9      | D-2       | 796 nm                                        | 118 nm             |
| 2-6 (Invention)  | C-9     | D-12      | 796 nm                                        | 118 nm             |

It is evident from this data that pyrrolotriazole couplers such as C-9 form improved infrared dyes (further shifted into the infrared) compared to conventional phenolic couplers known to the art. Furthermore, the amount of bathochromic shift with a hue-shifting developer is much greater with a pyrrolotriazole coupler compared to phenol couplers. This is unexpected, and results in much improved infrared dyes.

### Example 3

To demonstrate that the invention is capable of forming an infrared image that can be scanned, a coating identical in composition to Sample 1-2 was loaded into a 35 mm camera and exposed to a scene. The film sample was then processed thermally for 18 seconds at 161° C. Following removal of the silver, the film was scanned with a NIKON LS-2000 film scanner. This scanner, in addition to scanning in red, green, and blue channels, is also capable of scanning in the infrared. The output of the infrared channel was acquired into a personal computer using ADOBE PHOTOSHOP software, and subsequently printed to a thermal printer thus providing a hardcopy image of the original scene.

### MULTILAYER PHOTOGRAPHIC EXAMPLES

Processing conditions are as described in the examples. The following components are used in the examples:

Silver salt dispersion SS-1:

A stirred reaction vessel was charged with 480 g of lime processed gelatin and 5.6 l of distilled water. A solution containing 0.7 M silver nitrate was prepared (Solution A). A solution containing 0.7 M benzotriazole and 0.7 M NaOH was prepared (Solution B). The mixture in the reaction vessel was adjusted to a pAg of 7.25 and a pH of 8.00 by additions of Solution B, nitric acid, and sodium hydroxide as needed.

Solution A was added with vigorous mixing to the kettle at 38 cc/minute, and the pAg was maintained at 7.25 by a simultaneous addition of solution B. This process was continued until the quantity of silver nitrate added to the vessel was 3.54 M, at which point the flows were stopped and the mixture was concentrated by ultrafiltration. The resulting silver salt dispersion contained fine particles of silver benzotriazole.

### Silver salt dispersion SS-2:

A stirred reaction vessel was charged with 480 g of lime processed gelatin and 5.6 l of distilled water. A solution containing 0.7 M silver nitrate was prepared (Solution A). A solution containing 0.7 M 1-phenyl-5-mercaptopotetrazole and 0.7 M NaOH was also prepared (Solution B). The mixture in the reaction vessel was adjusted to a pAg of 7.25 and a pH of 8.00 by additions of Solution B, nitric acid, and sodium hydroxide as needed.

Solution A was added to the kettle at 19.6 cc/minute, and the pAg was maintained at 7.25 by a simultaneous addition of solution B. This process was continued until the 3.54 moles of silver nitrate had been added to the vessels, at which point the flows were stopped and mixture was concentrated by ultrafiltration. The resulting silver salt dispersion contained fine particles of the silver salt of 1-phenyl-5-mercaptopotetrazole.

### Melt former MF-1 dispersion:

A dispersion of salicylanilide was prepared by the method of ball milling. To a total 20 g sample was added 3.0 gm salicylanilide solid, 0.20 g polyvinyl pyrrolidone, 0.20 g TRITON X-200 surfactant, 1.0 g gelatin, 15.6 g distilled water, and 20 ml of zirconia beads. The slurry was ball milled for 48 hours. Following milling, the zirconia beads were removed by filtration. The slurry was refrigerated prior to use. For preparations on a larger scale, the salicylanilide was media-milled to give a final dispersion containing 30% Salicylanilide, with 4% TRITON X 200 surfactant and 4% polyvinyl pyrrolidone added relative to the weight of Salicylanilide. In some cases the dispersion was diluted with water to 25% Salicylanilide or gelatin (5% of total) was added and the concentration of Salicylanilide adjusted to 25%. If gelatin is added, biocide (KATHON) is also added.

### Developer D-17 Dispersion:

A slurry was milled in water containing developer D-17 and Olin 10G as a surfactant. The Olin 10G was added at a level of 10% by weight of the D-17. To the resulting slurry was added water and dry gelatin in order to bring the final concentrations to 13% D-17 and 4% gelatin. The gelatin was allowed to swell by mixing the components at 15° C. for 90 minutes. After this swelling process, the gelatin was dissolved by bringing the mixture to 40° C. for 10 minutes, followed by cooling the chill set the dispersion.



### Developer D-2 Dispersion:

A slurry was milled in water containing developer D-2 at a concentration of 10% by weight of the total slurry and Triton TX-200 as a surfactant. The Triton TX-200 was added at a level of 20% by weight of the D-2. The slurry was milled

**51**

on a roller mill using 1.8 mm Zirconia beads as the milling media.



Developer D-12 Dispersion:

A slurry was milled in water containing developer D-3 at a concentration of 10% by weight of the total slurry and Triton TX-200 as a surfactant. The Triton TX-200 was added at a level of 20% by weight of the D-3. The slurry was milled on a roller mill using 1.8 mm Zirconia beads as the milling media.

**52**

-continued



D-12 25 Coupler Dispersion CC-1:

An oil based coupler dispersion was prepared by conventional means containing coupler C-9 at 6% and gelatin at 6%. Coupler solvent tricresyl phosphate was included at a weight ratio of 1:1 relative to coupler C-9.

Coupler Dispersion MC-1:

A coupler dispersion was prepared by conventional means containing coupler M-1 at 5.5% and gelatin at 8%. The dispersion contained coupler solvents tricresyl phosphate and CS-1 at weight ratios of 0.8 and 0.2 relative to the coupler M-1, respectively.

35 C-9



M-1



An oil based coupler dispersion was prepared by conventional means containing coupler Y-1 at 6% and gelatin at 6%. Coupler solvent CS-2 was included at a weight ratio of 1:1 relative to coupler Y-1.



-continued

Y-1 DYE-2

10  
15  
20DYE-3  
CS-225  
30  
35HAR-1  
40  
45AF-1  
50

DYE-1

AF-2  
5560  
65



The multilayer structure as shown in Table 5 below was coated on a polyethylene terephthalate support. The coating was accomplished using an extrusion hopper that applied each layer in an indecent process. The coating from Table 5 is the comparative multilayer coating, labeled coating ML-C-1.

TABLE 5

| Overcoat                                  |        |                  |
|-------------------------------------------|--------|------------------|
| Gelatin                                   | 1.2960 | g/m <sup>2</sup> |
| Silicone Polymer DC-200 (Dow Corning)     | 0.0389 |                  |
| Matte Beads                               | 0.1134 |                  |
| Dye- 1 (UV)                               | 0.0972 |                  |
| FC-135 Fluorinated Surfactant             | 0.1058 |                  |
| HAR-1                                     | 0.5108 |                  |
| <u>Fast Yellow</u>                        |        |                  |
| Gelatin                                   | 1.9980 | g/m <sup>2</sup> |
| SS-1                                      | 0.1512 |                  |
| SS-2                                      | 0.1512 |                  |
| YC-1                                      | 0.2160 |                  |
| MF-1                                      | 0.5184 |                  |
| D-17                                      | 0.5184 |                  |
| Yellow Sens. Emulsion: 3.5 × 0.128 micron | 0.4860 |                  |
| AF-6                                      | 0.0079 |                  |
| <u>Slow Yellow</u>                        |        |                  |
| Gelatin                                   | 2.7540 | g/m <sup>2</sup> |
| SS-1                                      | 0.2376 |                  |
| SS-2                                      | 0.2376 |                  |
| YC-1                                      | 0.3780 |                  |
| MF-1                                      | 0.5832 |                  |
| D-17                                      | 0.5832 |                  |
| Yellow Sens. Emulsion: 1.5 × 0.129 micron | 0.2160 |                  |
| Yellow Sens. Emulsion: 0.6 × 0.139 micron | 0.0756 |                  |
| Yellow Sens. Emulsion: 0.5 × 0.13 micron  | 0.1512 |                  |
| Yellow Sens. Emulsion: 0.55 × 0.08 micron | 0.1512 |                  |
| AF-6                                      | 0.0096 |                  |
| <u>Interlayer 2</u>                       |        |                  |
| Gelatin                                   | 1.0800 | g/m <sup>2</sup> |
| AF-1                                      | 0.0022 |                  |
| DYE-2                                     | 0.0864 |                  |
| <u>Fast Magenta</u>                       |        |                  |
| Gelatin                                   | 1.7820 | g/m <sup>2</sup> |

TABLE 5-continued

|      |                                             |                         |
|------|---------------------------------------------|-------------------------|
| AF-3 |                                             |                         |
| 5    | SS-1                                        | 0.1512                  |
|      | SS-2                                        | 0.1512                  |
|      | MC-1                                        | 0.2160                  |
|      | MF-1                                        | 0.2160                  |
|      | D-17                                        | 0.2160                  |
|      | Magenta Sens. Emulsion: 2.1 × 0.131 micron  | 0.4860                  |
|      | AF-6                                        | 0.0079                  |
|      | <u>Mid Magenta</u>                          |                         |
| 10   | Gelatin                                     | 1.1340 g/m <sup>2</sup> |
|      | SS-1                                        | 0.1188                  |
|      | SS-2                                        | 0.1188                  |
|      | MC-1                                        | 0.1944                  |
|      | MF-1                                        | 0.1188                  |
| 15   | D-17                                        | 0.1188                  |
|      | Magenta Sens. Emulsion: 1.37 × 0.119 micron | 0.0648                  |
|      | Magenta Sens. Emulsion: 0.6 × 0.139 micron  | 0.1728                  |
|      | AF-6                                        | 0.0039                  |
|      | <u>Slow Magenta</u>                         |                         |
| 20   | Gelatin                                     | 1.1340 g/m <sup>2</sup> |
|      | SS-1                                        | 0.1188                  |
|      | SS-2                                        | 0.1188                  |
|      | MC-1                                        | 0.1944                  |
|      | MF-1                                        | 0.1188                  |
|      | D-17                                        | 0.1188                  |
|      | Magenta Sens. Emulsion: 0.5 × 0.13 micron   | 0.1080                  |
|      | Magenta Sens. Emulsion: 0.55 × 0.08 micron  | 0.1404                  |
| 25   | AF-6                                        | 0.0049                  |
|      | <u>Interlayer 1</u>                         |                         |
| 30   | Gelatin                                     | 1.0800 g/m <sup>2</sup> |
|      | AF-1                                        | 0.0022                  |
|      | <u>Fast Cyan</u>                            |                         |
| 35   | Gelatin                                     | 2.2140 g/m <sup>2</sup> |
|      | SS-1                                        | 0.1512                  |
|      | SS-2                                        | 0.1512                  |
|      | CC-1                                        | 0.2592                  |
|      | MF-1                                        | 0.5184                  |
|      | D-17                                        | 0.5184                  |
|      | Cyan Sens. Emulsion: 2.3 × 0.13 micron      | 0.4860                  |
|      | AF-6                                        | 0.0079                  |
|      | <u>Mid Cyan</u>                             |                         |
| 40   | Gelatin                                     | 1.7280 g/m <sup>2</sup> |
|      | SS-1                                        | 0.1188                  |
|      | SS-2                                        | 0.1188                  |
|      | CC-1                                        | 0.2322                  |
|      | MF-1                                        | 0.2916                  |
|      | D-17                                        | 0.2916                  |
|      | Cyan Sens. Emulsion: 1.37 × 0.119 micron    | 0.1512                  |
|      | Cyan Sens. Emulsion: 0.6 × 0.139 micron     | 0.1512                  |
| 45   | AF-6                                        | 0.0039                  |
|      | <u>Slow Cyan</u>                            |                         |
| 50   | Gelatin                                     | 1.7280 g/m <sup>2</sup> |
|      | SS-1                                        | 0.1188                  |
|      | SS-2                                        | 0.1188                  |
|      | CC-1                                        | 0.2322                  |
|      | MF-1                                        | 0.2916                  |
|      | D-17                                        | 0.2916                  |
|      | Cyan Sens. Emulsion: 0.55 × 0.08 micron     | 0.1512                  |
|      | Cyan Sens. Emulsion: 0.5 × 0.13 micron      | 0.1512                  |
| 55   | AF-6                                        | 0.0049                  |
|      | <u>AHU-01</u>                               |                         |
| 60   | DYE-3                                       | 0.0432 g/m <sup>2</sup> |
|      | Gelatin                                     | 1.6200                  |
|      | AF-2                                        | 0.0076                  |
|      | AF-3                                        | 0.2700                  |
|      | AF-4                                        | 0.0005                  |
|      | AF-5                                        | 0.0008                  |
|      | AF-1                                        | 0.0022                  |

65 The inventive coating is the same as the comparative coating, except that the Fast Yellow and Slow Yellow layers are substituted with the formulation listed in Table 6. The inventive multilayer coating is labeled coating ML-I-1.

TABLE 6

| Fast Yellow                               |        | g/m <sup>2</sup> |
|-------------------------------------------|--------|------------------|
| Gelatin                                   | 1.9980 |                  |
| SS-1                                      | 0.1512 |                  |
| SS-2                                      | 0.1512 |                  |
| CC-1                                      | 0.1620 |                  |
| MF-1                                      | 0.5184 |                  |
| D-2                                       | 0.2700 |                  |
| D-12                                      | 0.3780 |                  |
| Yellow Sens. Emulsion: 3.5 x 0.128 micron | 0.4860 |                  |
| AF-6                                      | 0.0079 |                  |
| Slow Yellow                               |        |                  |
| Gelatin                                   | 2.7540 | g/m <sup>2</sup> |
| SS-1                                      | 0.2376 |                  |
| SS-2                                      | 0.2376 |                  |
| CC-1                                      | 0.2700 |                  |
| MF-1                                      | 0.5832 |                  |
| D-2                                       | 0.2940 |                  |
| D-12                                      | 0.4000 |                  |
| Yellow Sens. Emulsion: 1.5 x 0.129 micron | 0.2160 |                  |
| Yellow Sens. Emulsion: 0.6 x 0.139 micron | 0.0756 |                  |
| Yellow Sens. Emulsion: 0.5 x 0.13 micron  | 0.1512 |                  |
| Yellow Sens. Emulsion: 0.55 x 0.08 micron | 0.1512 |                  |
| AF-6                                      | 0.0096 |                  |

Coatings ML-C-1 and ML-I-1 were exposed with white light filtered to simulate a color temperature of 5500 K for the exposure levels as listed in Table 7. After exposure, the coatings were processed for 18" at 157° C. in a roller transport drum thermal processor, and then subjected to the bleach and fix processes typically used during C-41 development. At that point, spectra of the resulting coatings were obtained to determine the level of dye formation associated with the various color records. This information is shown in Table 7.

TABLE 7

| Exposure    | Optical density |        |                |        |
|-------------|-----------------|--------|----------------|--------|
|             | Coating ML-C-1  |        | Coating ML-I-1 |        |
| Level (lux) | 465 nm          | 780 nm | 465 nm         | 780 nm |
| 0.25        | 0.58            | 0.09   | 0.31           | 0.42   |
| 1.58        | 0.99            | 0.15   | 0.44           | 0.71   |
| 10.00       | 1.63            | 0.27   | 0.63           | 1.07   |
| 63.10       | 2.26            | 0.33   | 0.77           | 1.35   |

Table 7 shows that the comparative coating shows very little activity in the IR region represented by 780 nm wavelength, while showing very strong activity in the blue region represented by 465 nm wavelength. Meanwhile, the inventive coating shows the opposite trend of low activity in the blue region with high activity in the IR region, indicating that it is successfully converting visual information in a scene into IR information for detection and reproduction of the image. This represents a working example of a film in which information in the blue channel is read out by the formation of infrared density. The fact that the activity of the systems is not zero in the spectral regions that are not intended to produce image information (780 nm for coating ML-C-1 and 465 nm for coating ML-I-1) is a result of the fact that in all photographic systems there are so called unwanted absorptions that lead to undesired density in some spectral regions.

The invention has been described in detail with particular reference to certain preferred embodiments thereof, but it will be understood that variations and modifications can be effected within the spirit and scope of the invention.

What is claimed is:

1. A light-sensitive color photothermographic imaging element comprising at least one pyrrolotriazole coupler in

reactive association with a developer, or developer Visor that liberates a developing agent, wherein the pyrrolotriazole coupler and the developing agent have the property that it is capable of forming a reaction product that is an infrared dye with a  $\lambda_{\text{max}}$  of greater than 700 nm.

2. The light-sensitive color photothermographic element of claim 1, wherein the pyrrolotriazole coupler has one of the following structures (IV) to (VII):

(IV)



(V)



(VI)



(VII)



wherein R<sup>7</sup>, R<sup>8</sup> and R<sup>9</sup> each represents a hydrogen atom or a substituent group, Y is a hydrogen atom or a group which is removable by the coupling reaction with a developing agent oxidant, and Z is hydrogen atom or a group capable of being released upon color development.

3. The light-sensitive color photothermographic element of claim 1, wherein either R<sup>7</sup> or R<sup>8</sup> is an electron attractive group, and R<sup>9</sup> provides ballast for the coupler.

4. The light-sensitive color photothermographic element of claim 1, wherein the pyrrolotriazole coupler has the following structure:

(VIII)



wherein R<sup>10</sup> and R<sup>11</sup> each represents an alkyl group or an aryl group; R<sup>12</sup>, R<sup>13</sup> and R<sup>14</sup> each represents a hydrogen atom, an alkyl group or an aryl group; W represents a non-metallic atomic group necessary to form a saturated ring; R<sup>15</sup> represents a substituent; Y represents a

**59**

coupling-off group; and Z represents a hydrogen atom or a group capable of being released upon color development.

5. The light-sensitive color photothermographic element of claim 1, wherein the pyrrolotriazole coupler has the following structure:



(IX)  
10  
15  
20  
25

wherein R<sup>17</sup> is an alkyl group; R<sup>a</sup>, R<sup>b</sup>, R<sup>c</sup>, R<sup>a'</sup>, R<sup>b'</sup>, and R<sup>c'</sup>, each are a atom or an alkyl group; R<sup>a</sup> and R<sup>b</sup>, and R<sup>a'</sup> and R<sup>b'</sup>, may respectively bond together to form a ring; R<sup>16</sup> is a hydrogen atom or an alkyl group, and X is heterocyclic group, a substituted amino group, or an aryl group.

6. The light-sensitive color photothermographic element of claim 1, wherein the pyrrolotriazole coupler is selected from the group consisting of:



C-1  
35  
40  
45  
50  
55  
60  
65



**60**  
-continued

C-3



C-4



C-5

61

-continued



62

-continued

C-9



20 7. The light-sensitive color photothermographic element of claim 1, wherein the developer precursor liberates a developer is a phenylenediamine compound having 2,6 ortho substitution.

8. The light sensitive color photothermographic element  
25 of claim 1, wherein the developer precursor liberates a  
developer represented by the following structure:



wherein  $R^1$ ,  $R^2$ ,  $R^3$ ,  $R^4$ ,  $R^5$  and  $R^6$  which can be the same or different are individually H, alkyl, substituted alkyl, alkenyl, substituted alkenyl, aryl, substituted aryl, halogen, cyano, hydroxy, alkoxy, substituted alkoxy, aryloxy, substituted aryloxy, amino, substituted amino, alkylcarbonamido, substituted alkylcarbonamido, arylcarbonamido, substituted arylcarbonamido, alkylsulfonamido, arylsulfonamido, substituted alkylsulfonamido, substituted arylsulfonamido, or sulfamyl or wherein at least two of  $R^1$ ,  $R^2$ ,  $R^3$  and  $R^4$  together further form a substituted or unsubstituted carbocyclic or heterocyclic ring structure; wherein  $R^3$  and  $R^5$  and/or  $R^4$  and  $R^6$  can be connected to form a substituted or unsubstituted carbocyclic or heterocyclic ring structure; except that neither  $R^1$  nor  $R^2$  can be H.

9. The light sensitive photothermographic element of claim 8, wherein the developer precursor liberates a developer represented by the following structure:



wherein  $R^1$  and  $R^2$  are as described above.

**10.** The light sensitive color photothermographic element of claim 1, wherein the element comprises a red-light-sensitive-layer unit, a green-light-sensitive layer unit and a blue-light-sensitive layer unit, wherein at least one layer unit has in reactive association the dye forming coupler and the blocked developer of claim 1.

**11.** The light sensitive color photothermographic element of claim 8 wherein the developer has the following structure:



wherein R<sub>1</sub> and R<sub>2</sub> is independently an alkyl or hydrogen substituent, optionally both hydrogen, and W<sub>1</sub> and W<sub>2</sub> represents an optional substituted or unsubstituted 5 or 6-membered cycloaliphatic ring on one or both sides or the above structure.

**12.** The light sensitive color photothermographic element of claim 1, wherein the element comprises a red light sensitive layer unit, a green light sensitive layer unit and a blue light sensitive layer unit and wherein all three layer units have in reactive association an independently selected dye forming coupler and an independently selected blocked developer, wherein the dye coupler is different in each layer unit and the developing agent is different in at least two layer units.

**13.** The light sensitive color photothermographic element of claim 1 wherein the element comprises a red light sensitive layer unit, a green light sensitive layer unit and a blue light sensitive layer unit and wherein all three layer units have in reactive association an independently selected dye forming coupler and an independently selected blocked developer, wherein the dye-forming couplers are the same in two of the layer units and wherein the blocked developer is different in said two layer units.

**14.** The element of claim 1, wherein said blocked developer and coupler is in reactive association with the red light sensitive color layer unit.

**15.** The color photographic element of claim 1, wherein the element is capable, after imagewise exposure, of being developed by heat treatment.

**16.** The color photographic element of claim 1, wherein the element is capable, after imagewise exposure, of development by treatment with base either by contacting the element with a pH controlling solution or by contacting the element with a pH controlling laminate.

**17.** The color photothermographic element of claim 1, wherein the color photographic element has a red light

sensitive silver halide layer unit and a first blocked coupling developer, a green light sensitive silver halide layer unit and a second blocked coupling developer and a blue light sensitive silver halide layer unit having a third blocked coupling developer.

**18.** A method of processing an imagewise exposed photothermographic element comprising a plurality of recording layer units, which method comprises thermally developing the imagewise exposed photothermographic element to form an image and then scanning the element to form an electronic image representation of the developed image in the element, wherein at least one image recording layer in at least one of the recording layer units comprises an infrared dye that is the reaction product of a pyrrolotriazole coupler and a developer, or developer precursor that liberates a developer, wherein the infrared dye has a  $\lambda_{\text{max}}$  of greater than 700 nm.

**19.** The method according to claim 18 further comprising digitizing an electronic image representation formed from the imagewise exposed, developed, and scanned photographic element to form a digital image.

**20.** The method according to claim 18 comprising the step of modifying a first electronic image representation formed from the imagewise exposed, developed, and scanned photographic element to form a second electronic image representation.

**21.** The method according to claim 18 comprising storing, transmitting, printing, or displaying an electronic image representation of an image derived from the imagewise exposed, developed, and scanned photographic element.

**22.** The method according to claim 21, wherein said electronic image representation is a digital image.

**23.** The method according to claim 21, wherein the method further comprises a printing step selected from the group consisting of electrophotography; inkjet; thermal dye sublimation; and CRT or LED printing to sensitized photographic paper.

**24.** The method according to claim 18 wherein said at least one image recording layer in the photothermographic element further comprises a light-sensitive silver halide emulsion and a non-light sensitive silver salt oxidizing agent.

**25.** The method according to claim 18 wherein the developing is accomplished in a dry state without the application of aqueous solutions.

**26.** The method according to claim 18 wherein the total amount of color masking coupler, the total amount of permanent Dmin adjusting dyes, and the permanent antihalation density, in blue, green and red density, is controlled so that the overall Dmin of the film minimizes the overall scanning noise during scanning.

**27.** A method according to claim 18 wherein said scanning occurs after partial desilvering of said element.

\* \* \* \* \*

UNITED STATES PATENT AND TRADEMARK OFFICE  
**CERTIFICATE OF CORRECTION**

PATENT NO. : 6,599,684 B2  
DATED : July 29, 2003  
INVENTOR(S) : James H. Reynolds, Leif P. Olson, Wojciech K. Slusarek and David H. Levy

Page 1 of 1

It is certified that error appears in the above-identified patent and that said Letters Patent is hereby corrected as shown below:

Column 57, line 68 through Column 58, line 5,

Claim 1, should read:

1. A light-sensitive color photothermographic imaging element comprising at least one pyrrolotriazole coupler in reactive association with a developer, or developer precursor that liberates a developing agent, wherein the pyrrolotriazole coupler and the developing agent have the property that it is capable of forming a reaction product that is an infrared dye with a  $\lambda_{max}$  of greater than 700 nm.

Signed and Sealed this

Second Day of March, 2004



JON W. DUDAS  
*Acting Director of the United States Patent and Trademark Office*